# EUROPEAN PATENT SPECIFICATION

(11) **EP 4 530 724 B1**
(45) Date of publication and mention of the grant of the patent: **17.06.2026**
(21) Application number: 24159917.4
(22) Date of filing: 27.02.2024
(51) Int. Cl.: G03G 5/05, G03G 5/147

(54) **ELECTROPHOTOGRAPHIC PHOTORECEPTOR, PROCESS CARTRIDGE, AND IMAGE FORMING APPARATUS**
ELEKTROPHOTOGRAPHISCHER PHOTOREZEPTOR, PROZESSKARTUSCHE UND BILDERZEUGUNGSVORRICHTUNG
PHOTORÉCEPTEUR ÉLECTROPHOTOGRAPHIQUE, CARTOUCHE DE TRAITEMENT ET APPAREIL DE FORMATION D'IMAGE

(30) Priority: 27.09.2023 JP 2023165025
(43) Date of publication of application: 02.04.2025
(73) Proprietor: FUJIFILM Business Innovation Corp., Minato-ku Tokyo (JP)
(72) Inventor: KUSANO, Keisuke, Ebina-shi, Kanagawa (JP); IDE, Kenta, Ebina-shi, Kanagawa (JP); KOBAYASHI, Hiroko, Ebina-shi, Kanagawa (JP); KIGOSHI, Yoichi, Ebina-shi, Kanagawa (JP); OYAMADA, Yuki, Ebina-shi, Kanagawa (JP)
(74) Representative: Kurig, Thomas

(56) References cited:
- JP-A- 2007 213 051
- JP-B2- 5 664 342

## Description

### BACKGROUND OF THE INVENTION

### (i) Field of the Invention

The present invention relates to an electrophotographic photoreceptor, a process cartridge, and an image forming apparatus.

### (ii) Description of Related Art

The formation of an image by an electrophotographic method is performed, for example, by charging a surface of a photoreceptor to form an electrostatic charge image on the surface of the photoreceptor according to image information, developing the electrostatic charge image with a developer containing a toner to form a toner image, and transferring and fixing the toner image to a surface of a recording medium.

JP2010-217598A discloses "an image forming unit including a photoreceptor, a charging unit that charges a surface of the photoreceptor, a developing unit that develops an electrostatic latent image formed on the surface of the photoreceptor with a developer by irradiating the surface with exposure light, to form a developer image on the surface of the photoreceptor, and a cleaning unit that is brought into pressure contact with the surface of the photoreceptor to remove the residual developer on the surface of the photoreceptor, in which an outermost layer of the photoreceptor has a Martens hardness value of 175 to 196 N/mm², an elastic deformation rate of 35% to 48%, and a static friction coefficient of 0.535 or less".

JP2014-209221A discloses "an electrophotographic photoreceptor including at least a photosensitive layer on a conductive support, in which the photosensitive layer contains a polyarylate resin having a carboxylic acid terminal value of 100 µ equivalent/g or greater and 500 µ equivalent/g or less and a triphenylamine compound".

JP 5 664342 B2 discloses an electrophotographic photosensitive member comprising a specific polyester resin as a binder resin in a photosensitive layer, a process cartridge and an image forming apparatus including the electrophotographic photosensitive member.

JP 2007 213051 A discloses an electrophotographic photoreceptor having a photosensitive layer on a conductive support, and an image forming apparatus using the same.

### SUMMARY OF THE INVENTION

An object of the present disclosure is to provide an electrophotographic photoreceptor that has excellent abrasion resistance and is capable of suppressing abnormal discharge even in a case of being charged with only a DC voltage as compared with a case where the electrophotographic photoreceptor has an outermost layer containing a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by less than 5% or greater than 12%. The present invention is defined in the appended claims. The following disclosure serves a better understanding of the present invention.

Specific means for achieving the above-described object includes the following aspects.
<1> According to a first aspect of the present disclosure, there is provided an electrophotographic photoreceptor including: an outermost layer that contains a charge transport material and a binder resin, in which the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by a range of 5% or greater and 12% or less.
<2> According to a second aspect of the present disclosure, there is provided the electrophotographic photoreceptor according to <1>, in which a content ratio (polyester resin P_{A}:Polycarbonate resin P_{B}) of the polyester resin P_{A} to the polycarbonate resin P_{B} may be in a range of 7:3 to 3:7 in terms of a mass.
<3> According to a third aspect of the present disclosure, there is provided the electrophotographic photoreceptor according to <2>, in which the content ratio (polyester resin P_{A}:Polycarbonate resin P_{B}) of the polyester resin P_{A} to the polycarbonate resin P_{B} may be in a range of 7:3 to 5:5 in terms of the mass.
<4> According to a fourth aspect of the present disclosure, there is provided the electrophotographic photoreceptor according to any one of <1> to <3>, in which the polyester resin PA may include a polyester resin having a dicarboxylic acid unit (A) represented by Formula (A) and a diol unit (B) represented by Formula (B).
<5> According to a fifth aspect of the present disclosure, there is provided the electrophotographic photoreceptor according to any one of <1> to <4>, in which the polycarbonate resin P_{B} may include a polycarbonate resin having a constitutional unit represented by Formula (PCA) and a constitutional unit represented by Formula (PCB).
<6> According to a sixth aspect of the present disclosure, there is provided a process cartridge including: the electrophotographic photoreceptor according to any one of <1> to <5>, in which the process cartridge is attachable to and detachable from an image forming apparatus.
<7> According to a seventh aspect of the present disclosure, there is provided an image forming apparatus including: the electrophotographic photoreceptor according to any one of <1> to <5>; a charging device that comes into direct contact with a surface of the electrophotographic photoreceptor and applies only a DC voltage to charge the surface of the electrophotographic photoreceptor; an electrostatic latent image forming device that forms an electrostatic latent image on the charged surface of the electrophotographic photoreceptor; a developing device that develops the electrostatic latent image formed on the surface of the electrophotographic photoreceptor with a developer containing a toner to form a toner image; and a transfer device that transfers the toner image to a surface of a recording medium.
<8> According to an eighth aspect of the present disclosure, there is provided the image forming apparatus according to <7>, in which the charging device may include a charging member that charges the surface of the electrophotographic photoreceptor and a DC voltage application unit that applies only the DC voltage to the charging member, and a voltage applied to the charging member from the DC voltage application unit is -700 V or greater and -300 V or less.

According to <1>, <4>, or <5>, it is possible to provide an electrophotographic photoreceptor that has excellent abrasion resistance and is capable of suppressing abnormal discharge even in a case of being charged with only a DC voltage as compared with a case where the electrophotographic photoreceptor has an outermost layer containing a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by less than 5% or greater than 12%.

According to <2> or <3>, it is possible to provide an electrophotographic photoreceptor that has excellent abrasion resistance and is capable of suppressing abnormal discharge even in a case of being charged with only a DC voltage as compared with a case where polyester resin P_{A}:polycarbonate resin P_{B} is out of the range of 7:3 to 3:7 in terms of the mass.

According to <6>, <7>, or <8>, it is possible to provide a process cartridge or an image forming apparatus, including an electrophotographic photoreceptor that has excellent abrasion resistance and is capable of suppressing abnormal discharge even in a case of being charged with only a DC voltage as compared with a case where the electrophotographic photoreceptor has an outermost layer containing a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by less than 5% or greater than 12%.

### BRIEF DESCRIPTION OF THE DRAWINGS

Exemplary embodiment(s) of the present invention will be described in detail based on the following figures, wherein:
Fig. 1 is a partial cross-sectional view showing an example of a layer configuration of an electrophotographic photoreceptor according to the present exemplary embodiment;
Fig. 2 is a partial cross-sectional view showing an example of a layer configuration of an electrophotographic photoreceptor according to the present exemplary embodiment;
Fig. 3 is a schematic configuration view showing an example of an image forming apparatus according to the present exemplary embodiment; and
Fig. 4 is a schematic configuration view showing another example of an image forming apparatus according to the present exemplary embodiment.

### DETAILED DESCRIPTION OF THE INVENTION

Hereinafter, exemplary embodiments of the present disclosure will be described. The following descriptions and examples merely illustrate the exemplary embodiments, and do not limit the scope of the exemplary embodiments.

In the present disclosure, a numerical range shown using "to" indicates a range including numerical values described before and after "to" as a minimum value and a maximum value.

In a numerical range described in a stepwise manner in the present disclosure, an upper limit value or a lower limit value described in a certain numerical range may be replaced with an upper limit value or a lower limit value in another numerical range described in a stepwise manner. Further, in a numerical range described in the present disclosure, an upper limit value or a lower limit value described in the numerical range may be replaced with a value shown in examples.

In the present disclosure, in a case where an exemplary embodiment is described with reference to drawings, the configuration of the exemplary embodiment is not limited to the configuration shown in the drawings. In addition, the sizes of members in each drawing are conceptual and the relative relation in the sizes between the members is not limited thereto.

In the present disclosure, each component may include a plurality of kinds of substances corresponding to each component. In the present disclosure, in a case where a plurality of kinds of substances corresponding to each component in a composition are present, the amount of each component in the composition indicates the total amount of the plurality of kinds of substances present in the composition unless otherwise specified.

In the present disclosure, each component may include a plurality of kinds of particles corresponding to each component. In a case where a plurality of kinds of particles corresponding to each component are present in a composition, the particle diameter of each component indicates the value of a mixture of the plurality of kinds of particles present in the composition, unless otherwise specified.

In the present disclosure, the term "(meth)acryl" may denote any of "acryl" or "methacryl".

In the present disclosure, an alkyl group is any of linear, branched, or cyclic unless otherwise specified.

### <Electrophotographic Photoreceptor>

An electrophotographic photoreceptor according to the present disclosure includes an outermost layer that contains a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by a range of 5% or greater and 12% or less.

Hereinafter, "electrophotographic photoreceptor" will also be simply referred to as "photoreceptor".

In order to improve the abrasion resistance of the photoreceptor, the development of a technique of using a resin with high durability to the outermost layer of the photoreceptor, for example, a resin with an elastic deformation rate X_{A} of 53.0% or greater is progressing.

Meanwhile, since the resin with an elastic deformation rate X_{A} of 53.0% or greater has high durability, the surface of the photoreceptor having an outermost layer that contains the resin is difficult to scrape, and discharge products are likely to be accumulated on the surface of the photoreceptor. In particular, in a case of the photoreceptor in which the outermost layer includes a photosensitive layer containing a charge transport material, a local abnormal discharge phenomenon occurs in a case where the photoreceptor is charged by a DC charging method using only a DC voltage, and thus the image quality of the output image may be degraded.

As a result of examination on a technique of suppressing abnormal discharge even in a case where a photoreceptor is charged with only a DC voltage while maintaining the abrasion resistance, the present inventors have found the configuration of the photoreceptor according to the present disclosure.

That is, the present inventors have found that the abnormal discharge can be suppressed even in a case where the photoreceptor is charged with only a DC voltage while maintaining the abrasion resistance, by using a polyester resin P_{A} and a polycarbonate resin P_{B} as the binder resin contained in the outermost layer together with the charge transport material and by setting a difference (elastic deformation rate X_{A} - elastic deformation rate X_{B}) in elastic deformation rate between the polyester resin P_{A} and the polycarbonate resin P_{B}, which has high durability, to be in a range of 5% or greater and 12% or less.

Hereinafter, "abnormal discharge in a case where the photoreceptor is charged with only a DC voltage" will also be simply referred to as "abnormal discharge".

Further, in a case where the photoreceptor according to the present disclosure undergoes actual machine traveling, an uneven shape is formed on the outermost layer due to a difference in the elastic deformation rate between the two kinds of resins. In a case where the developer contains a silicone component, the silicone component in the developer is appropriately accumulated on recesses of the outermost layer so that the apparent friction coefficient is decreased, and thus the cleaning performance in the surface of the photoreceptor is improved in some cases.

### <Layer Configuration>

Hereinafter, the layer configurations of the photoreceptor according to the present exemplary embodiment will be described.

Fig. 1 is a partial cross-sectional view schematically showing an example of a layer configuration of a photoreceptor according to the present exemplary embodiment. A photoreceptor 10A shown in Fig. 1 includes a lamination type photosensitive layer. The photoreceptor 10A has a structure in which an undercoat layer 2, a charge generation layer 3, and a charge transport layer 4 are laminated in this order on a conductive substrate 1, and the charge generation layer 3 and the charge transport layer 4 constitute a photosensitive layer 5 (so-called function separation type photosensitive layer). The photoreceptor 10A may include an interlayer (not shown) between the undercoat layer 2 and the charge generation layer 3.

Fig. 2 is a partial cross-sectional view schematically showing an example of a layer configuration of a photoreceptor according to the present exemplary embodiment. A photoreceptor 10B shown in Fig. 2 includes a single layer type photosensitive layer. The photoreceptor 10B has a structure in which the undercoat layer 2 and the photosensitive layer 5 are laminated in this order on the conductive substrate 1. The photoreceptor 10B may include an interlayer (not shown) between the undercoat layer 2 and the photosensitive layer 5.

### [Outermost Layer]

Since the outermost layer contains a charge transport material and a binder resin, the outermost layer corresponds to a charge transport layer in the lamination type photosensitive layer or a single layer type photosensitive layer in the single layer type photosensitive layer described above.

### [Binder Resin]

In the outermost layer, the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by a range of 5% or greater and 12% or less.

Here, a difference (elastic deformation rate X_{A} - elastic deformation rate X_{B}) in elastic deformation rate between the polyester resin P_{A} and the polycarbonate resin P_{B} is 5% or greater and 12% or less and, for example, more preferably 7% or greater and 10% or less.

The elastic deformation rates of the polyester resin P_{A} and the polycarbonate resin P_{B} are determined in the following manner.

Here, the elastic deformation rate is defined as "elastic deformation rate = elastic deformation amount/total deformation amount" by dividing the total deformation amount in a case where a load is applied to a measuring object into an elastic deformation amount and a plastic deformation amount. Specifically, first, a resin layer having a thickness of 5 µm which is formed of only a resin is obtained as a measuring object. Further, the elastic deformation rate is calculated by measuring the indentation depth and "indentation depth - stress curve" of the resin layer using Nanoindenter SA2 (manufactured by MTS), a DCM head, and an equilateral triangular pyramid indenter made of diamond. More specifically, an elastic deformation rate R of the resin layer is calculated by using the following equation under a measurement condition that the indentation depth set to 500 nm in an environment of a temperature of 24°C and a humidity of 50% is defined as Dmax (nm) and the indentation depth in a case where the load is completely removed is defined as D1 (nm). The calculated elastic deformation rate R is defined as the elastic deformation rate of the resin constituting the resin layer.$Elastic deformation rate R = \left(Dmax-D1\right) / Dmax$

### (Polyester Resin P_{A})

Hereinafter, the polyester resin P_{A} having an elastic deformation rate X_{A} of 53.0 % or greater will be described.

The polyester resin P_{A} is not particularly limited as long as the elastic deformation rate X_{A} is 53.0% or greater.

The elastic deformation rate X_{A} of the polyester resin P_{A} is 53.0% or greater and, for example, more preferably 58.0% or greater.

Further, the upper limit value of the elastic deformation rate X_{A} of the polyester resin P_{A} is, for example, 60.0%.

It is preferable that the polyester resin P_{A} includes, for example, a polyester resin having a dicarboxylic acid unit (A) represented by Formula (A) and a diol unit (B) represented by Formula (B).

Hereinafter, the polyester resin having a dicarboxylic acid unit (A) represented by Formula (A) and a diol unit (B) represented by Formula (B) will be referred to as "polyester resin (1)".

In Formula (A), Ar^{A1} and Ar^{A2} each independently represent an aromatic ring that may have a substituent, L^{A} represents a single bond or a divalent linking group, and n^{A1} represents 0, 1, or 2.

In Formula (B), Ar^{B1} and Ar^{B2} each independently represent an aromatic ring that may have a substituent, L^{B} represents a single bond, an oxygen atom, a sulfur atom, or -C(Rb¹)(Rb²)-, n^{B1} represents 0, 1, or 2. Rb¹ and Rb² each independently represent a hydrogen atom, an alkyl group having 1 or more and 20 or less carbon atoms, an aryl group having 6 or more and 12 or less carbon atoms, or an aralkyl group having 7 or more and 20 or less carbon atoms, and Rb¹ and Rb² may be bonded to each other to form a cyclic alkyl group.

The polyester resin (1) may have other dicarboxylic acid units in addition to the dicarboxylic acid unit (A). The polyester resin (1) may have other diol units in addition to the diol unit (B).

The dicarboxylic acid unit (A) is a constitutional unit represented by Formula (A).

In Formula (A), Ar^{A1} and Ar^{A2} each independently represent an aromatic ring that may have a substituent, L^{A} represents a single bond or a divalent linking group, and n^{A1} represents 0, 1, or 2.

The aromatic ring as Ar^{A1} may be any of a monocycle or a polycycle. Examples of the aromatic ring include a benzene ring, a naphthalene ring, an anthracene ring, and a phenanthrene ring. Among these, for example, a benzene ring and a naphthalene ring are preferable.

The hydrogen atom on the aromatic ring as Ar^{A1} may be substituted with an alkyl group, an aryl group, an aralkyl group, an alkoxy group, an aryloxy group, a halogen atom, or the like. As the substituent in a case where the aromatic ring as Ar^{A1} is substituted, for example, an alkyl group having 1 or more and 10 or less carbon atoms, an aryl group having 6 or more and 12 or less carbon atoms, and an alkoxy group having 1 or more and 6 or less carbon atoms are preferable.

The aromatic ring of Ar^{A2} may be any of a monocycle or a polycycle. Examples of the aromatic ring include a benzene ring, a naphthalene ring, an anthracene ring, and a phenanthrene ring. Among these, for example, a benzene ring and a naphthalene ring are preferable.

The hydrogen atom on the aromatic ring as Ar^{A2} may be substituted with an alkyl group, an aryl group, an aralkyl group, an alkoxy group, an aryloxy group, a halogen atom, or the like. As the substituent in a case where the aromatic ring as Ar^{A2} is substituted, for example, an alkyl group having 1 or more and 10 or less carbon atoms, an aryl group having 6 or more and 12 or less carbon atoms, and an alkoxy group having 1 or more and 6 or less carbon atoms are preferable.

In a case where L^{A} represents a divalent linking group, examples of the divalent linking group include an oxygen atom, a sulfur atom, and -C(Ra¹)(Ra²)-. Here, Ra¹ and Ra² each independently represent a hydrogen atom, an alkyl group having 1 or more and 10 or less carbon atoms, an aryl group having 6 or more and 12 or less carbon atoms, or an aralkyl group having 7 or more and 20 or less carbon atoms, and Ra¹ and Ra² may be bonded to each other to form a cyclic alkyl group.

The alkyl group having 1 or more and 10 or less carbon atoms as Ra¹ and Ra² may be any of linear, branched, or cyclic. The number of carbon atoms of the alkyl group is, for example, preferably 1 or more and 6 or less, more preferably 1 or more and 4 or less, and still more preferably 1 or 2.

The aryl group having 6 or more and 12 or less carbon atoms as Ra¹ and Ra² may be any of a monocycle or a polycycle. The number of carbon atoms of the aryl group is, for example, preferably 6 or more and 10 or less and more preferably 6.

The alkyl group in the aralkyl group having 7 or more and 20 or less carbon atoms as Ra¹ and Ra² may be any of linear, branched, or cyclic. The number of carbon atoms of the alkyl group in the aralkyl group having 7 or more and 20 or less carbon atoms is, for example, preferably 1 or more and 4 or less, more preferably 1 or more and 3 or less, and still more preferably 1 or 2.

The aryl group in the aralkyl group having 7 or more and 20 or less carbon atoms as Ra¹ and Ra² may be any of a monocycle or a polycycle. The number of carbon atoms of the aryl group is, for example, preferably 6 or more and 10 or less and more preferably 6.

It is preferable that the dicarboxylic acid unit (A) includes, for example, at least one selected from the group consisting of a dicarboxylic acid unit (A1) represented by Formula (A1), a dicarboxylic acid unit (A2) represented by Formula (A2), a dicarboxylic acid unit (A3) represented by Formula (A3), and a dicarboxylic acid unit (A4) represented by Formula (A4). The dicarboxylic acid unit (A) includes, for example, more preferably at least one selected from the group consisting of a dicarboxylic acid unit (A2), a dicarboxylic acid unit (A3), and a dicarboxylic acid unit (A4) and still more preferably a dicarboxylic acid unit (A2).

In Formula (A1), n¹⁰¹ represents an integer of 0 or greater and 4 or less, and n¹⁰¹ pieces of Ra¹⁰¹'s each independently represent an alkyl group having 1 or more and 10 or less carbon atoms, an aryl group having 6 or more and 12 or less carbon atoms, or an alkoxy group having 1 or more and 6 or less carbon atoms.

n¹⁰¹ represents, for example, preferably 0, 1, or 2, more preferably 0 or 1, and still more preferably 0.

In Formula (A2), n²⁰¹ and n²⁰² each independently represent an integer of 0 or greater and 4 or less, and n²⁰¹ pieces of Ra²⁰¹'s and n²⁰² pieces of Ra²⁰²'s each independently represent an alkyl group having 1 or more and 10 or less carbon atoms, an aryl group having 6 or more and 12 or less carbon atoms, or an alkoxy group having 1 or more and 6 or less carbon atoms.
n²⁰¹ represents, for example, preferably 0, 1, or 2, more preferably 0 or 1, and still more preferably 0.
n²⁰² represents, for example, preferably 0, 1, or 2, more preferably 0 or 1, and still more preferably 0.

In Formula (A3), n³⁰¹ and n³⁰² each independently represent an integer of 0 or greater and 4 or less, and n³⁰¹ pieces of Ra³⁰¹'s and n³⁰² pieces of Ra³⁰²'s each independently represent an alkyl group having 1 or more and 10 or less carbon atoms, an aryl group having 6 or more and 12 or less carbon atoms, or an alkoxy group having 1 or more and 6 or less carbon atoms.
n³⁰¹ represents, for example, preferably 0, 1, or 2, more preferably 0 or 1, and still more preferably 0.
n³⁰² represents, for example, preferably 0, 1, or 2, more preferably 0 or 1, and still more preferably 0.

In Formula (A4), n⁴⁰¹ represents an integer of 0 or greater and 6 or less, and n⁴⁰¹ pieces of Ra⁴⁰¹'s each independently represent an alkyl group having 1 or more and 10 or less carbon atoms, an aryl group having 6 or more and 12 or less carbon atoms, or an alkoxy group having 1 or more and 6 or less carbon atoms.
n⁴⁰¹ represents, for example, preferably an integer of 0 or greater and 4 or less, more preferably 0, 1, or 2, and still more preferably 0.

The specific forms and the desired forms of Ra¹⁰¹ in Formula (A1), Ra²⁰¹ and Ra²⁰² in Formula (A2), Ra³⁰¹ and Ra³⁰² in Formula (A3), and Ra⁴⁰¹ in Formula (A4) are the same as each other, and hereinafter, Ra¹⁰¹, Ra²⁰¹, Ra²⁰², Ra³⁰¹, Ra³⁰², and Ra⁴⁰¹ will be collectively referred to as "Ra".

The alkyl group having 1 or more and 10 or less carbon atoms as Ra may be any of linear, branched, or cyclic. The number of carbon atoms of the alkyl group is, for example, preferably 1 or more and 6 or less, more preferably 1 or more and 4 or less, and still more preferably 1 or 2.

Examples of the linear alkyl group having 1 or more and 10 or less carbon atoms include a methyl group, an ethyl group, an n-propyl group, an n-butyl group, an n-pentyl group, an n-hexyl group, an n-heptyl group, an n-octyl group, an n-nonyl group, and an n-decyl group.

Examples of the branched alkyl group having 3 or more and 10 or less carbon atoms include an isopropyl group, an isobutyl group, a sec-butyl group, a tert-butyl group, an isopentyl group, a neopentyl group, a tert-pentyl group, an isohexyl group, a sec-hexyl group, a tert-hexyl group, an isoheptyl group, a sec-heptyl group, a tert-heptyl group, an isooctyl group, a sec-octyl group, a tert-octyl group, an isononyl group, a sec-nonyl group, a tert-nonyl group, an isodecyl group, a sec-decyl group, and a tert-decyl group.

Examples of the cyclic alkyl group having 3 or more and 10 or less carbon atoms include a cyclopropyl group, a cyclobutyl group, a cyclopentyl group, a cyclohexyl group, a cycloheptyl group, a cyclooctyl group, a cyclononyl group, a cyclodecyl group, and polycyclic (for example, bicyclic, tricyclic, or spirocyclic) alkyl groups to which these monocyclic alkyl groups are linked.

The aryl group having 6 or more and 12 or less carbon atoms as Ra may be any of a monocycle or a polycycle. The number of carbon atoms of the aryl group is, for example, preferably 6 or more and 10 or less and more preferably 6.

Examples of the aryl group having 6 or more and 12 or less carbon atoms include a phenyl group, a biphenyl group, a 1-naphthyl group, and a 2-naphthyl group.

The alkyl group in the alkoxy group having 1 or more and 6 or less carbon atoms as Ra may be any of linear, branched, or cyclic. The number of carbon atoms of the alkyl group in the alkoxy group having 1 or more and 6 or less carbon atoms is, for example, preferably 1 or more and 4 or less, more preferably 1 or more and 3 or less, and still more preferably 1 or 2.

Examples of the linear alkoxy group having 1 or more and 6 or less carbon atoms include a methoxy group, an ethoxy group, an n-propoxy group, an n-butoxy group, an n-pentyloxy group, and an n-hexyloxy group.

Examples of the branched alkoxy group having 3 or more and 6 or less carbon atoms include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, and a tert-hexyloxy group.

Examples of the cyclic alkoxy group having 3 or more and 6 or less carbon atoms include a cyclopropoxy group, a cyclobutoxy group, a cyclopentyloxy group, and a cyclohexyloxy group.

Hereinafter, dicarboxylic acid units (A1-1) to (A1-9) are shown as specific examples of the dicarboxylic acid unit (A1). The dicarboxylic acid unit (A1) is not limited thereto.

Hereinafter, dicarboxylic acid units (A2-1) to (A2-3) are shown as specific examples of the dicarboxylic acid unit (A2). The dicarboxylic acid unit (A2) is not limited thereto.

Hereinafter, dicarboxylic acid units (A3-1) and (A3-2) are shown as specific examples of the dicarboxylic acid unit (A3). The dicarboxylic acid unit (A3) is not limited thereto.

Hereinafter, dicarboxylic acid units (A4-1) to (A4-3) are shown as specific examples of the dicarboxylic acid unit (A4). The dicarboxylic acid unit (A4) is not limited thereto.

The polyester resin has, for example, preferably at least one selected from the group consisting of (A1-1), (A1-7), (A2-3), (A3-2), and (A4-3), more preferably at least one selected from the group consisting of (A2-3), (A3-2), and (A4-3), and still more preferably at least (A2-3) as the dicarboxylic acid unit (A).

The total mass proportion of the dicarboxylic acid units (A1) to (A4) in the polyester resin (1) is, for example, preferably 15% by mass or greater and 60% by mass or less.

In a case where the total mass proportion of the dicarboxylic acid units (A1) to (A4) is 15% by mass or greater, the abrasion resistance of the photosensitive layer is enhanced. From this viewpoint, the total mass proportion of the dicarboxylic acid units (A1) to (A4) is, for example, more preferably 20% by mass or greater and still more preferably 25% by mass or greater.

In a case where the total mass proportion of the dicarboxylic acid units (A1) to (A4) is 60% by mass or less, peeling of the photosensitive layer can be suppressed. From this viewpoint, the total mass proportion of the dicarboxylic acid units (A1) to (A4) is, for example, more preferably 55% by mass or less and still more preferably 50% by mass or less.

The dicarboxylic acid units (A1) to (A4) contained in the polyester resin (1) may be used alone or in combination of two or more kinds thereof.

Examples of other dicarboxylic acid units (A) in addition to the dicarboxylic acid units (A1) to (A4) include aliphatic dicarboxylic acid (such as oxalic acid, malonic acid, maleic acid, fumaric acid, citraconic acid, itaconic acid, glutaconic acid, succinic acid, alkenyl succinic acid, adipic acid, and sebacic acid) units, alicyclic dicarboxylic acid (such as cyclohexanedicarboxylic acid) units, and lower (for example, having 1 or more and 5 or less carbon atoms) alkyl ester units thereof. These dicarboxylic acid units contained in the polyester resin (1) may be used alone or in combination of two or more kinds thereof.

The dicarboxylic acid unit (A) contained in the polyester resin (1) may be used alone or in combination of two or more kinds thereof.

The diol unit (B) is a constitutional unit represented by Formula (B).

In Formula (B), Ar^{B1} and Ar^{B2} each independently represent an aromatic ring that may have a substituent, L^{B} represents a single bond, an oxygen atom, a sulfur atom, or -C(Rb¹)(Rb²)-, n^{B1} represents 0, 1, or 2. Rb¹ and Rb² each independently represent a hydrogen atom, an alkyl group having 1 or more and 20 or less carbon atoms, an aryl group having 6 or more and 12 or less carbon atoms, or an aralkyl group having 7 or more and 20 or less carbon atoms, and Rb¹ and Rb² may be bonded to each other to form a cyclic alkyl group.

The aromatic ring as Ar^{B1} may be any of a monocycle or a polycycle. Examples of the aromatic ring include a benzene ring, a naphthalene ring, an anthracene ring, and a phenanthrene ring. Among these, for example, a benzene ring and a naphthalene ring are preferable.

The hydrogen atom on the aromatic ring as Ar^{B1} may be substituted with an alkyl group, an aryl group, an aralkyl group, an alkoxy group, an aryloxy group, a halogen atom, or the like. As the substituent in a case where the aromatic ring as Ar^{B1} is substituted, for example, an alkyl group having 1 or more and 10 or less carbon atoms, an aryl group having 6 or more and 12 or less carbon atoms, and an alkoxy group having 1 or more and 6 or less carbon atoms are preferable.

The aromatic ring as Ar^{B2} may be any of a monocycle or a polycycle. Examples of the aromatic ring include a benzene ring, a naphthalene ring, an anthracene ring, and a phenanthrene ring. Among these, for example, a benzene ring and a naphthalene ring are preferable.

The hydrogen atom on the aromatic ring as Ar^{B2} may be substituted with an alkyl group, an aryl group, an aralkyl group, an alkoxy group, an aryloxy group, a halogen atom, or the like. As the substituent in a case where the aromatic ring as Ar^{B2} is substituted, for example, an alkyl group having 1 or more and 10 or less carbon atoms, an aryl group having 6 or more and 12 or less carbon atoms, and an alkoxy group having 1 or more and 6 or less carbon atoms are preferable.

The alkyl group having 1 or more and 20 or less carbon atoms as Rb¹ and Rb² may be linear, branched, or cyclic. The number of carbon atoms of the alkyl group is, for example, preferably 1 or more and 18 or less, more preferably 1 or more and 14 or less, and still more preferably 1 or more and 10 or less.

The aryl group having 6 or more and 12 or less carbon atoms as Rb¹ and Rb² may be any of a monocycle or a polycycle. The number of carbon atoms of the aryl group is, for example, preferably 6 or more and 10 or less and more preferably 6.

The alkyl group in the aralkyl group having 7 or more and 20 or less carbon atoms as Rb¹ and Rb² may be any of linear, branched, or cyclic. The number of carbon atoms of the alkyl group in the aralkyl group having 7 or more and 20 or less carbon atoms is, for example, preferably 1 or more and 4 or less, more preferably 1 or more and 3 or less, and still more preferably 1 or 2.

The aryl group in the aralkyl group having 7 or more and 20 or less carbon atoms as Rb¹ and Rb² may be any of a monocycle or a polycycle. The number of carbon atoms of the aryl group is, for example, preferably 6 or more and 10 or less and more preferably 6.

It is preferable that the diol unit (B) includes, for example, at least one selected from the group consisting of a diol unit (B1) represented by Formula (B 1), a diol unit (B2) represented by Formula (B2), a diol unit (B3) represented by Formula (B3), a diol unit (B4) represented by Formula (B4), a diol unit (B5) represented by Formula (B5), a diol unit (B6) represented by Formula (B6), a diol unit (B7) represented by Formula (B7), and a diol unit (B8) represented by Formula (B8).

The diol unit (B) includes, for example, more preferably at least one selected from the group consisting of a diol unit (B1) represented by Formula (B1), a diol unit (B2) represented by Formula (B2), a diol unit (B4) represented by Formula (B4), a diol unit (B5) represented by Formula (B5), and a diol unit (B6) represented by Formula (B6), still more preferably at least one selected from the group consisting of a diol unit (B1) represented by Formula (B1), a diol unit (B2) represented by Formula (B2), a diol unit (B5) represented by Formula (B5), and a diol unit (B6) represented by Formula (B6), even still more preferably at least one selected from the group consisting of a diol unit (B1) represented by Formula (B1), a diol unit (B2) represented by Formula (B2), and a diol unit (B6) represented by Formula (B6), and most preferably at least one selected from the group consisting of a diol unit (B1) represented by Formula (B1) and a diol unit (B2) represented by Formula (B2).

In Formula (B1), Rb¹⁰¹ represents a branched alkyl group having 4 or more and 20 or less carbon atoms, Rb²⁰¹ represents a hydrogen atom or an alkyl group having 1 or more and 3 or less carbon atoms, and Rb⁴⁰¹, Rb⁵⁰¹, Rb⁸⁰¹, and Rb⁹⁰¹ each independently represent a hydrogen atom, an alkyl group having 1 or more and 4 or less carbon atoms, an alkoxy group having 1 or more and 6 or less carbon atoms, or a halogen atom.

The number of carbon atoms of the branched alkyl group having 4 or more and 20 or less carbon atoms as Rb¹⁰¹ is, for example, preferably 4 or more and 16 or less, more preferably 4 or more and 12 or less, and still more preferably 4 or more and 8 or less. Specific examples of Rb¹⁰¹ include an isobutyl group, a sec-butyl group, a tert-butyl group, an isopentyl group, a neopentyl group, a tert-pentyl group, an isohexyl group, a sec-hexyl group, a tert-hexyl group, an isoheptyl group, a sec-heptyl group, a tert-heptyl group, an isooctyl group, a sec-octyl group, a tert-octyl group, an isononyl group, a sec-nonyl group, a tert-nonyl group, an isodecyl group, a sec-decyl group, a tert-decyl group, an isododecyl group, a sec-dodecyl group, a tert-dodecyl group, a tert-tetradecyl group, and a tert-pentadecyl group.

In Formula (B2), Rb¹⁰² represents a linear alkyl group having 4 or more and 20 or less carbon atoms, Rb²⁰² represents a hydrogen atom or an alkyl group having 1 or more and 3 or less carbon atoms, and Rb⁴⁰², Rb⁵⁰², Rb⁸⁰², and Rb⁹⁰² each independently represent a hydrogen atom, an alkyl group having 1 or more and 4 or less carbon atoms, an alkoxy group having 1 or more and 6 or less carbon atoms, or a halogen atom.

The number of carbon atoms of the linear alkyl group having 4 or more and 20 or less carbon atoms as Rb¹⁰² is, for example, preferably 4 or more and 16 or less, more preferably 4 or more and 12 or less, and still more preferably 4 or more and 8 or less. Specific examples of Rb¹⁰² include an n-butyl group, an n-pentyl group, an n-hexyl group, an n-heptyl group, an n-octyl group, an n-nonyl group, an n-decyl group, an n-undecyl group, an n-dodecyl group, a tridecyl group, an n-tetradecyl group, an n-pentadecyl group, an n-heptadecyl group, an n-octadecyl group, an n-nonadecyl group, and an n-icosyl group.

In Formula (B3), Rb¹¹³ and Rb²¹³ each independently represent a hydrogen atom, a linear alkyl group having 1 or more and 3 or less carbon atoms, an alkoxy group having 1 or more and 4 or less carbon atoms, or a halogen atom, d represents an integer of 7 or greater and 15 or less, and Rb⁴⁰³, Rb⁵⁰³, Rb⁸⁰³, and Rb⁹⁰³ each independently represent a hydrogen atom, an alkyl group having 1 or more and 4 or less carbon atoms, an alkoxy group having 1 or more and 6 or less carbon atoms, or a halogen atom.

The number of carbon atoms of the linear alkyl group having 1 or more and 3 or less carbon atoms as Rb¹¹³ and Rb²¹³ is, for example, preferably 1 or 2 and more preferably 1. Specific examples of such a group include a methyl group, an ethyl group, and an n-propyl group.

The alkyl group in the alkoxy group having 1 or more and 4 or less carbon atoms as Rb¹¹³ and Rb²¹³ may be linear, branched, or cyclic. The number of carbon atoms of the alkyl group in the alkoxy group having 1 or more and 4 or less carbon atoms is, for example, preferably 1 or more and 3 or less, more preferably 1 or 2, and still more preferably 1. Specific examples of such a group include a methoxy group, an ethoxy group, an n-propoxy group, an n-butoxy group, an isopropoxy group, an isobutoxy group, a sec-butoxy group, a tert-butoxy group, a cyclopropoxy group, and a cyclobutoxy group.

Examples of the halogen atom as Rb¹¹³ and Rb²¹³ include a fluorine atom, a chlorine atom, a bromine atom, and an iodine atom.

In Formula (B4), Rb¹⁰⁴ and Rb²⁰⁴ each independently represent a hydrogen atom, an alkyl group having 1 or more and 3 or less carbon atoms, and Rb⁴⁰⁴, Rb⁵⁰⁴, Rb⁸⁰⁴, and Rb⁹⁰⁴ each independently represent a hydrogen atom, an alkyl group having 1 or more and 4 or less carbon atoms, an alkoxy group having 1 or more and 6 or less carbon atoms, or a halogen atom.

The alkyl group having 1 or more and 3 or less carbon atoms as Rb¹⁰⁴ may be any of linear, branched, or cyclic. The number of carbon atoms of the alkyl group is, for example, preferably 1 or 2 and more preferably 1. Specific examples of Rb¹⁰⁴ include a methyl group, an ethyl group, an n-propyl group, an isopropyl group, and a cyclopropyl group.

In Formula (B5), Ar¹⁰⁵ represents an aryl group having 6 or more and 12 or less carbon atoms or an aralkyl group having 7 or more and 20 or less carbon atoms, Rb²⁰⁵ represents a hydrogen atom or an alkyl group having 1 or more and 3 or less carbon atoms, and Rb⁴⁰⁵, Rb⁵⁰⁵, Rb⁸⁰⁵, and Rb⁹⁰⁵ each independently represent a hydrogen atom, an alkyl group having 1 or more and 4 or less carbon atoms, an alkoxy group having 1 or more and 6 or less carbon atoms, or a halogen atom.

The aryl group having 6 or more and 12 or less carbon atoms as Ar¹⁰⁵ may be any of a monocycle or a polycycle. The number of carbon atoms of the aryl group is, for example, preferably 6 or more and 10 or less and more preferably 6.

The alkyl group in the aralkyl group having 7 or more and 20 or less carbon atoms as Ar¹⁰⁵ may be any of linear, branched, or cyclic. The number of carbon atoms of the alkyl group in the aralkyl group having 7 or more and 20 or less carbon atoms is, for example, preferably 1 or more and 4 or less, more preferably 1 or more and 3 or less, and still more preferably 1 or 2. The aryl group in the aralkyl group having 7 or more and 20 or less carbon atoms as Ar¹⁰⁵ may be any of a monocycle or a polycycle. The number of carbon atoms of the aryl group is, for example, preferably 6 or more and 10 or less and more preferably 6. Examples of the aralkyl group having 7 or more and 20 or less carbon atoms include a benzyl group, a phenylethyl group, a phenylpropyl group, a 4-phenylbutyl group, a phenylpentyl group, a phenylhexyl group, a phenylheptyl group, a phenyloctyl group, a phenylnonyl group, a naphthylmethyl group, a naphthylethyl group, an anthracenylmethyl group, and a phenyl-cyclopentylmethyl group.

In Formula (B6), Rb¹¹⁶ and Rb²¹⁶ each independently represent a hydrogen atom, a linear alkyl group having 1 or more and 3 or less carbon atoms, an alkoxy group having 1 or more and 4 or less carbon atoms, or a halogen atom, e represents an integer of 4 or greater and 6 or less, and Rb⁴⁰⁶, Rb⁵⁰⁶, Rb⁸⁰⁶, and Rb⁹⁰⁶ each independently represent a hydrogen atom, an alkyl group having 1 or more and 4 or less carbon atoms, an alkoxy group having 1 or more and 6 or less carbon atoms, or a halogen atom.

The number of carbon atoms of the linear alkyl group having 1 or more and 3 or less carbon atoms as Rb¹¹⁶ and Rb²¹⁶ is, for example, preferably 1 or 2 and more preferably 1. Specific examples of such a group include a methyl group, an ethyl group, and an n-propyl group.

The alkyl group in the alkoxy group having 1 or more and 4 or less carbon atoms as Rb¹¹⁶ and Rb²¹⁶ may be linear, branched, or cyclic. The number of carbon atoms of the alkyl group in the alkoxy group having 1 or more and 4 or less carbon atoms is, for example, preferably 1 or more and 3 or less, more preferably 1 or 2, and still more preferably 1. Specific examples of such a group include a methoxy group, an ethoxy group, an n-propoxy group, an n-butoxy group, an isopropoxy group, an isobutoxy group, a sec-butoxy group, a tert-butoxy group, a cyclopropoxy group, and a cyclobutoxy group.

Examples of the halogen atom as Rb¹¹⁶ and Rb²¹⁶ include a fluorine atom, a chlorine atom, a bromine atom, and an iodine atom.

In Formula (B7), Rb⁴⁰⁷, Rb⁵⁰⁷, Rb⁸⁰⁷, and Rb⁹⁰⁷ each independently represent a hydrogen atom, an alkyl group having 1 or more and 4 or less carbon atoms, an alkoxy group having 1 or more and 6 or less carbon atoms, or a halogen atom.

In Formula (B8), Rb⁴⁰⁸, Rb⁵⁰⁸, Rb⁸⁰⁸, and Rb⁹⁰⁸ each independently represent a hydrogen atom, an alkyl group having 1 or more and 4 or less carbon atoms, an alkoxy group having 1 or more and 6 or less carbon atoms, or a halogen atom.

The specific forms and the desired forms of Rb²⁰¹ in Formula (B1), Rb²⁰² in Formula (B2), Rb²⁰⁴ in Formula (B4), and Rb²⁰⁵ in Formula (B5) are the same as each other, and hereinafter, Rb²⁰¹, Rb²⁰², Rb²⁰⁴, and Rb²⁰⁵ will be collectively referred to as "Rb²⁰⁰".

The alkyl group having 1 or more and 3 or less carbon atoms as Rb²⁰⁰ may be any of linear, branched, or cyclic. The number of carbon atoms of the alkyl group is, for example, preferably 1 or 2 and more preferably 1.

The alkyl group having 1 or more and 3 or less carbon atoms includes a methyl group, an ethyl group, an n-propyl group, an isopropyl group, and a cyclopropyl group.

The specific forms and the desired forms of Rb⁴⁰¹ in Formula (B1), Rb⁴⁰² in Formula (B2), Rb⁴⁰³ in Formula (B3), Rb⁴⁰⁴ in Formula (B4), Rb⁴⁰⁵ in Formula (B5), Rb⁴⁰⁶ in Formula (B6), Rb⁴⁰⁷ in Formula (B7), and Rb⁴⁰⁸ in Formula (B8) are the same as each other, and hereinafter, Rb⁴⁰¹, Rb⁴⁰², Rb⁴⁰³, Rb⁴⁰⁴, Rb⁴⁰⁵, Rb⁴⁰⁶, Rb⁴⁰⁷, and Rb⁴⁰⁸ will be collectively referred to as "Rb⁴⁰⁰".

The alkyl group having 1 or more and 4 or less carbon atoms as Rb⁴⁰⁰ may be any of linear, branched, or cyclic. The number of carbon atoms of the alkyl group is, for example, preferably 1 or more and 3 or less, more preferably 1 or 2, and still more preferably 1.

Examples of the linear alkyl group having 1 or more and 4 or less carbon atoms include a methyl group, an ethyl group, an n-propyl group, and an n-butyl group.

Examples of the branched alkyl group having 3 or 4 carbon atoms include an isopropyl group, an isobutyl group, a sec-butyl group, and a tert-butyl group.

Examples of the cyclic alkyl group having 3 or 4 carbon atoms include a cyclopropyl group and a cyclobutyl group.

The alkyl group in the alkoxy group having 1 or more and 6 or less carbon atoms as Rb⁴⁰⁰ may be any of linear, branched, or cyclic. The number of carbon atoms of the alkyl group in the alkoxy group having 1 or more and 6 or less carbon atoms is, for example, preferably 1 or more and 4 or less, more preferably 1 or more and 3 or less, and still more preferably 1 or 2.

Examples of the linear alkoxy group having 1 or more and 6 or less carbon atoms include a methoxy group, an ethoxy group, an n-propoxy group, an n-butoxy group, an n-pentyloxy group, and an n-hexyloxy group.

Examples of the branched alkoxy group having 3 or more and 6 or less carbon atoms include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, and a tert-hexyloxy group.

Examples of the cyclic alkoxy group having 3 or more and 6 or less carbon atoms include a cyclopropoxy group, a cyclobutoxy group, a cyclopentyloxy group, and a cyclohexyloxy group.

Examples of the halogen atom as Rb⁴⁰⁰ include a fluorine atom, a chlorine atom, a bromine atom, and an iodine atom.

The specific forms and the desired forms of Rb⁵⁰¹ in Formula (B1), Rb⁵⁰² in Formula (B2), Rb⁵⁰³ in Formula (B3), Rb⁵⁰⁴ in Formula (B4), Rb⁵⁰⁵ in Formula (B5), Rb⁵⁰⁶ in Formula (B6), Rb⁵⁰⁷ in Formula (B7), and Rb⁵⁰⁸ in Formula (B8) are the same as each other, and hereinafter, Rb⁵⁰¹, Rb⁵⁰², Rb⁵⁰³, Rb⁵⁰⁴, Rb⁵⁰⁵, Rb⁵⁰⁶, Rb⁵⁰⁷, and Rb⁵⁰⁸ will be collectively referred to as "Rb⁵⁰⁰".

The alkyl group having 1 or more and 4 or less carbon atoms as Rb⁵⁰⁰ may be any of linear, branched, or cyclic. The number of carbon atoms of the alkyl group is, for example, preferably 1 or more and 3 or less, more preferably 1 or 2, and still more preferably 1.

Examples of the linear alkyl group having 1 or more and 4 or less carbon atoms include a methyl group, an ethyl group, an n-propyl group, and an n-butyl group.

Examples of the branched alkyl group having 3 or 4 carbon atoms include an isopropyl group, an isobutyl group, a sec-butyl group, and a tert-butyl group.

Examples of the cyclic alkyl group having 3 or 4 carbon atoms include a cyclopropyl group and a cyclobutyl group.

The alkyl group in the alkoxy group having 1 or more and 6 or less carbon atoms as Rb⁵⁰⁰ may be any of linear, branched, or cyclic. The number of carbon atoms of the alkyl group in the alkoxy group having 1 or more and 6 or less carbon atoms is, for example, preferably 1 or more and 4 or less, more preferably 1 or more and 3 or less, and still more preferably 1 or 2.

Examples of the linear alkoxy group having 1 or more and 6 or less carbon atoms include a methoxy group, an ethoxy group, an n-propoxy group, an n-butoxy group, an n-pentyloxy group, and an n-hexyloxy group.

Examples of the branched alkoxy group having 3 or more and 6 or less carbon atoms include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, and a tert-hexyloxy group.

Examples of the cyclic alkoxy group having 3 or more and 6 or less carbon atoms include a cyclopropoxy group, a cyclobutoxy group, a cyclopentyloxy group, and a cyclohexyloxy group.

Examples of the halogen atom as Rb⁵⁰⁰ include a fluorine atom, a chlorine atom, a bromine atom, and an iodine atom.

The specific forms and the desired forms of Rb⁸⁰¹ in Formula (B1), Rb⁸⁰² in Formula (B2), Rb⁸⁰³ in Formula (B3), Rb⁸⁰⁴ in Formula (B4), Rb⁸⁰⁵ in Formula (B5), Rb⁸⁰⁶ in Formula (B6), Rb⁸⁰⁷ in Formula (B7), and Rb⁸⁰⁸ in Formula (B8) are the same as each other, and hereinafter, Rb⁸⁰¹, Rb⁸⁰², Rb⁸⁰³, Rb⁸⁰⁴, Rb⁸⁰⁵, Rb⁸⁰⁶, Rb⁸⁰⁷, and Rb⁸⁰⁸ will be collectively referred to as "Rb⁸⁰⁰".

The alkyl group having 1 or more and 4 or less carbon atoms as Rb⁸⁰⁰ may be any of linear, branched, or cyclic. The number of carbon atoms of the alkyl group is, for example, preferably 1 or more and 3 or less, more preferably 1 or 2, and still more preferably 1.

Examples of the linear alkyl group having 1 or more and 4 or less carbon atoms include a methyl group, an ethyl group, an n-propyl group, and an n-butyl group.

Examples of the branched alkyl group having 3 or 4 carbon atoms include an isopropyl group, an isobutyl group, a sec-butyl group, and a tert-butyl group.

Examples of the cyclic alkyl group having 3 or 4 carbon atoms include a cyclopropyl group and a cyclobutyl group.

The alkyl group in the alkoxy group having 1 or more and 6 or less carbon atoms as Rb⁸⁰⁰ may be any of linear, branched, or cyclic. The number of carbon atoms of the alkyl group in the alkoxy group having 1 or more and 6 or less carbon atoms is, for example, preferably 1 or more and 4 or less, more preferably 1 or more and 3 or less, and still more preferably 1 or 2.

Examples of the linear alkoxy group having 1 or more and 6 or less carbon atoms include a methoxy group, an ethoxy group, an n-propoxy group, an n-butoxy group, an n-pentyloxy group, and an n-hexyloxy group.

Examples of the branched alkoxy group having 3 or more and 6 or less carbon atoms include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, and a tert-hexyloxy group.

Examples of the cyclic alkoxy group having 3 or more and 6 or less carbon atoms include a cyclopropoxy group, a cyclobutoxy group, a cyclopentyloxy group, and a cyclohexyloxy group.

Examples of the halogen atom as Rb⁸⁰⁰ include a fluorine atom, a chlorine atom, a bromine atom, and an iodine atom.

The specific forms and the desired forms of Rb⁹⁰¹ in Formula (B1), Rb⁹⁰² in Formula (B2), Rb⁹⁰³ in Formula (B3), Rb⁹⁰⁴ in Formula (B4), Rb⁹⁰⁵ in Formula (B5), Rb⁹⁰⁶ in Formula (B6), Rb⁹⁰⁷ in Formula (B7), and Rb⁹⁰⁸ in Formula (B8) are the same as each other, and hereinafter, Rb⁹⁰¹, Rb⁹⁰², Rb⁹⁰³, Rb⁹⁰⁴, Rb⁹⁰⁵, Rb⁹⁰⁶, Rb⁹⁰⁷, and Rb⁹⁰⁸ will be collectively referred to as "Rb⁹⁰⁰".

The alkyl group having 1 or more and 4 or less carbon atoms as Rb⁹⁰⁰ may be any of linear, branched, or cyclic. The number of carbon atoms of the alkyl group is, for example, preferably 1 or more and 3 or less, more preferably 1 or 2, and still more preferably 1.

Examples of the linear alkyl group having 1 or more and 4 or less carbon atoms include a methyl group, an ethyl group, an n-propyl group, and an n-butyl group.

Examples of the branched alkyl group having 3 or 4 carbon atoms include an isopropyl group, an isobutyl group, a sec-butyl group, and a tert-butyl group.

Examples of the cyclic alkyl group having 3 or 4 carbon atoms include a cyclopropyl group and a cyclobutyl group.

The alkyl group in the alkoxy group having 1 or more and 6 or less carbon atoms as Rb⁹⁰⁰ may be any of linear, branched, or cyclic. The number of carbon atoms of the alkyl group in the alkoxy group having 1 or more and 6 or less carbon atoms is, for example, preferably 1 or more and 4 or less, more preferably 1 or more and 3 or less, and still more preferably 1 or 2.

Examples of the linear alkoxy group having 1 or more and 6 or less carbon atoms include a methoxy group, an ethoxy group, an n-propoxy group, an n-butoxy group, an n-pentyloxy group, and an n-hexyloxy group.

Examples of the branched alkoxy group having 3 or more and 6 or less carbon atoms include an isopropoxy group, an isobutoxy group, a sec-butoxy group, a tert-butoxy group, an isopentyloxy group, a neopentyloxy group, a tert-pentyloxy group, an isohexyloxy group, a sec-hexyloxy group, and a tert-hexyloxy group.

Examples of the cyclic alkoxy group having 3 or more and 6 or less carbon atoms include a cyclopropoxy group, a cyclobutoxy group, a cyclopentyloxy group, and a cyclohexyloxy group.

Examples of the halogen atom as Rb⁹⁰⁰ include a fluorine atom, a chlorine atom, a bromine atom, and an iodine atom.

Hereinafter, diol units (B1-1) to (B1-6) are shown as specific examples of the diol unit (B1). The diol unit (B1) is not limited thereto.

Hereinafter, diol units (B2-1) to (B2-11) are shown as specific examples of the diol unit (B2). The diol unit (B2) is not limited thereto.

Hereinafter, diol units (B3-1) to (B3-4) are shown as specific examples of the diol unit (B3). The diol unit (B3) is not limited thereto.

Hereinafter, diol units (B4-1) to (B4-7) are shown as specific examples of the diol unit (B4). The diol unit (B4) is not limited thereto.

Hereinafter, diol units (B5-1) to (B5-6) are shown as specific examples of the diol unit (B5). The diol unit (B5) is not limited thereto.

Hereinafter, diol units (B6-1) to (B6-4) are shown as specific examples of the diol unit (B6). The diol unit (B6) is not limited thereto.

Hereinafter, diol units (B7-1) to (B7-3) are shown as specific examples of the diol unit (B7). The diol unit (B7) is not limited thereto.

Hereinafter, diol units (B8-1) to (B8-3) are shown as specific examples of the diol unit (B8). The diol unit (B8) is not limited thereto.

The diol unit (B) contained in the polyester resin (1) may be used alone or in combination of two or more kinds thereof.

The mass proportion of the diol unit (B) in the polyester resin (1) is, for example, preferably 25% by mass or greater and 80% by mass or less.

In a case where the mass proportion of the diol unit (B) is 25% by mass or greater, peeling of the photosensitive layer can be further suppressed. From this viewpoint, the mass proportion of the diol unit (B) is, for example, more preferably 30% by mass or greater and still more preferably 35% by mass or greater.

In a case where the mass proportion of the diol unit (B) is 80% by mass or less, the solubility in a coating solution for forming the photosensitive layer is maintained, and thus the abrasion resistance can be improved. From this viewpoint, the mass proportion of the diol unit (B) is, for example, more preferably 75% by mass or less and still more preferably 70% by mass or less.

Examples of other diol units in addition to the diol unit (B) include aliphatic diol (such as ethylene glycol, diethylene glycol, triethylene glycol, propylene glycol, butanediol, hexanediol, and neopentyl glycol) units and alicyclic diol (such as cyclohexanediol, cyclohexanedimethanol, and hydrogenated bisphenol A) units. These diol units contained in the polyester resin (1) may be used alone or in combination of two or more kinds thereof.

A terminal of the polyester resin (1) may be sealed or modified with a terminal-sealing agent, a molecular weight modifier, or the like used in a case of the production. Examples of the terminal-sealing agent or the molecular weight modifier include monohydric phenol, monovalent acid chloride, monohydric alcohol, and monovalent carboxylic acid.

Examples of the monohydric phenol include phenol, o-cresol, m-cresol, p-cresol, o-ethylphenol, m-ethylphenol, p-ethylphenol, o-propylphenol, m-propylphenol, p-propylphenol, o-tert-butylphenol, m-tert-butylphenol, p-tert-butylphenol, pentylphenol, hexylphenol, octylphenol, nonylphenol, a 2,6-dimethylphenol derivative, a 2-methylphenol derivative, o-phenylphenol, m-phenylphenol, p-phenylphenol, o-methoxyphenol, m-methoxyphenol, p-methoxyphenol, 2,3,5-trimethylphenol, 2,3,6-trimethylphenol, 2,3-xylenol, 2,4-xylenol, 2,5-xylenol, 2,6-xylenol, 3,4-xylenol, 3,5-xylenol, 2-phenyl-2-(4-hydroxyphenyl)propane, 2-phenyl-2-(2-hydroxyphenyl)propane, and 2-phenyl-2-(3-hydroxyphenyl)propane.

Examples of the monovalent acid chloride include monofunctional acid halides such as benzoyl chloride, benzoic acid chloride, methanesulfonyl chloride, phenylchloroformate, acetic acid chloride, butyric acid chloride, octyl acid chloride, benzenesulfonyl chloride, benzenesulfinyl chloride, sulfinyl chloride, benzene phosphonyl chloride, and substituents thereof.

Examples of the monohydric alcohol include methanol, ethanol, n-propanol, isopropanol, n-butanol, 2-butanol, pentanol, hexanol, dodecyl alcohol, stearyl alcohol, benzyl alcohol, and phenethyl alcohol.

Examples of the monovalent carboxylic acid include acetic acid, propionic acid, octanoic acid, cyclohexanecarboxylic acid, benzoic acid, toluic acid, phenylacetic acid, p-tert-butylbenzoic acid, and p-methoxyphenylacetic acid.

The weight-average molecular weight of the polyester resin (1) is, for example, preferably 30,000 or greater and 300,000 or less, more preferably 40,000 or greater and 250,000 or less, and still more preferably 50,000 or greater and 200,000 or less.

The molecular weight of the polyester resin (1) is a molecular weight measured by gel permeation chromatography (GPC) in terms of polystyrene. The GPC is carried out by using tetrahydrofuran as an eluent.

The polyester resin (1) can be obtained by polycondensing a monomer providing a dicarboxylic acid unit (A), a monomer providing a diol unit (B), and other monomers as necessary using a method of the related art. Examples of the method of polycondensing monomers include an interfacial polymerization method, a solution polymerization method, and a melt polymerization method. The interfacial polymerization method is a polymerization method of mixing a divalent carboxylic acid halide dissolved in an organic solvent that is incompatible with water and dihydric alcohol dissolved in an alkali aqueous solution to obtain polyester. Examples of documents related to the interfacial polymerization method include W. M. EARECKSON, J. Poly. Sci., XL399, 1959, and JP1965-1959B. Since the interfacial polymerization method enables the reaction to proceed faster than the reaction carried out by the solution polymerization method and also enables suppression of hydrolysis of the divalent carboxylic acid halide, as a result, a high-molecular-weight polyester resin can be obtained.

### (Polycarbonate Resin P_{B})

Hereinafter, the polycarbonate resin P_{B} will be described.

The polycarbonate resin P_{B} is not particularly limited as long as the difference in elastic deformation rate (elastic deformation rate X_{A} - elastic deformation rate X_{B}) between the polycarbonate resin P_{B} and the polyester resin P_{A} used in combination is in a range of 5% or greater and 12% or less.

It is preferable that the polycarbonate resin P_{B} includes, for example, a polycarbonate resin having a constitutional unit represented by Formula (PCA) and a constitutional unit represented by Formula (PCB).

The polycarbonate resin having a constitutional unit represented by Formula (PCA) and a constitutional unit represented by Formula (PCB) will be simply referred to as a polycarbonate resin (2).

In Formula (PCA), R^{P1} and R^{P2} each independently represent a hydrogen atom, a halogen atom, an alkyl group having 1 or more and 6 or less carbon atoms, a cycloalkyl group having 5 or more and 7 or less carbon atoms, or an aryl group having 6 or more and 12 or less carbon atoms.

In Formula (PCB), R^{P3} and R^{P4} each independently represent a hydrogen atom, a halogen atom, an alkyl group having 1 or more and 6 or less carbon atoms, a cycloalkyl group having 5 or more and 7 or less carbon atoms, or an aryl group having 6 or more and 12 or less carbon atoms. X^{P1} represents a phenylene group, a biphenylene group, a naphthylene group, a linear or branched alkylene group, or a cycloalkylene group.

Examples of the alkyl group represented by R^{P1}, R^{P2}, R^{P3}, and R^{P4} in Formulae (PCA) and (PCB) include a linear or branched alkyl group having 1 or more and 6 or less carbon atoms (for example, preferably 1 or more and 3 or less carbon atoms).

Specific examples of the linear alkyl group include a methyl group, an ethyl group, an n-propyl group, an n-butyl group, an n-pentyl group, and an n-hexyl group.

Specific examples of the branched alkyl group include an isopropyl group, an isobutyl group, a sec-butyl group, a tert-butyl group, an isopentyl group, a neopentyl group, a tert-pentyl group, an isohexyl group, a sec-hexyl group, and a tert-hexyl group.

Among these, for example, a lower alkyl group such as a methyl group or an ethyl group is preferable as the alkyl group.

Examples of the cycloalkyl group represented by R^{P1}, R^{P2} R^{P3}, and R^{P4} in Formulae (PCA) and (PCB) include cyclopentyl, cyclohexyl, and cycloheptyl.

Examples of the aryl group represented by R^{P1}, R^{P2}, R^{P3}, and R^{P4} in Formulae (PCA) and (PCB) include a phenyl group, a naphthyl group, and a biphenylyl group.

Examples of the alkylene group represented by X^{P1} in Formulae (PCA) and (PCB) include a linear or branched alkylene group having 1 or more and 12 or less carbon atoms (for example, preferably 1 or more and 6 or less carbon atoms and more preferably 1 or more and 3 or less carbon atoms).

Specific examples of the linear alkylene group include a methylene group, an ethylene group, an n-propylene group, an n-butylene group, an n-pentylene group, an n-hexylene group, an n-heptylene group, an n-octylene group, an n-nonylene group, an n-decylene group, an n-undecylene group, and an n-dodecylene group.

Specific examples of the branched alkylene group include an isopropylene group, an isobutylene group, a sec-butylene group, a tert-butylene group, an isopentylene group, a neopentylene group, a tert-pentylene group, an isohexylene group, a sec-hexylene group, a tert-hexylene group, an isoheptylene group, a sec-heptylene group, a tert-heptylene group, an isooctylene group, a sec-octylene group, a tert-octylene group, an isononylene group, a sec-nonylene group, a tert-nonylene group, an isodecylene group, a sec-decylene group, a tert-decylene group, an isoundecylene group, a sec-undecylene group, a tert-undecylene group, a neoundecylene group, an isododecylene group, a sec-dodecylene group, a tert-dodecylene group, and a neododecylene group.

Among these, preferred examples of the alkylene group include a lower alkyl group such as a methylene group, an ethylene group, or a butylene group.

Examples of the cycloalkylene group represented by X^{P1} in Formulae (PCA) and (PCB) include a cycloalkylene group having 3 or more and 12 or less carbon atoms (for example, preferably 3 or more and 10 or less carbon atoms and more preferably 5 or more and 8 or less carbon atoms).

Specific examples of the cycloalkyl group include a cyclopropyl group, a cyclopentyl group, a cyclohexyl group, a cyclooctyl group, and a cyclododecanyl group.

Among these, for example, a cyclohexyl group is preferable as the cycloalkyl group.

Further, each substituent represented by R^{P1} R^{P2}, R^{P3}, R^{P4}, or X^{P1} in Formulae (PCA) and (PCB) includes a group further having a substituent. Examples of the substituent include a halogen atom (such as a fluorine atom or a chlorine atom), an alkyl group (such as an alkyl group having 1 or more and 6 or less carbon atoms), a cycloalkyl group (such as a cycloalkyl group having 5 or more and 7 or less carbon atoms), an alkoxy group (such as an alkoxy group having 1 or more and 4 or less carbon atoms), and an aryl group (such as a phenyl group, a naphthyl group, or a biphenylyl group).

In Formula (PCA), R^{P1} and R^{P2} each independently represent, for example, preferably a hydrogen atom or an alkyl group having 1 or more and 6 or less carbon atoms and more preferably a hydrogen atom.

In Formula (PCB), it is preferable that R^{P3} and R^{P4} each independently represent, for example, a hydrogen atom or an alkyl group having 1 or more and 6 or less carbon atoms and that X^{P1} represents an alkylene group or a cycloalkylene group.

Specific examples of the polycarbonate resin (2) include the followings, but the present disclosure is not limited thereto. Further, in the exemplary compounds, pm and pn denote a copolymerization ratio.

Here, the content ratio (copolymerization ratio) of the structural unit represented by Formula (PCA) in the polycarbonate resin (2) may be, for example, in a range of 5% by mole or greater and 95% by mole or less with respect to all the structural units constituting the polycarbonate resin, and for example, preferably in a range of 5% by mole or greater and 50% by mole or less and more preferably in a range of 15% by mole or greater and 30% by mole or less from the viewpoint of suppressing the density unevenness of an image with graininess.

Specifically, pm and pn in the above-described exemplary compounds of the polycarbonate resin (2) denote a copolymerization ratio (molar ratio), and the copolymerization ratio between pm and pn (pm:pn) is, for example, preferably in a range of 95:5 to 5:95, more preferably in a range of 50:50 to 5:95, and still more preferably in a range of 15:85 to 30:70.

From the viewpoint of further suppressing abnormal discharge while maintaining the abrasion resistance, the content ratio of the polyester resin P_{A} to the polycarbonate resin P_{B} (polyester resin P_{A}:polycarbonate resin P_{B}) in the outermost layer is, for example, preferably in a range of 7:3 to 3:7 and more preferably in a range of 7:3 to 5:5 in terms of the mass.

### [Charge Transport Material]

Examples of the charge transport material include the same materials as the materials for the charge transport material in the charge transport layer described below.

Hereinafter, each member and each layer other than the outermost layer of the electrophotographic photoreceptor according to the present exemplary embodiment will be described in detail. Further, the reference numerals will not be provided.

### [Conductive Substrate]

· Examples of the conductive substrate include metal plates containing metals (such as aluminum, copper, zinc, chromium, nickel, molybdenum, vanadium, indium, gold, and platinum) or alloys (such as stainless steel), metal drums, and metal belts. Further, examples of the conductive substrate include paper, a resin film, a belt, and the like obtained by being coated, vapor-deposited or laminated with a conductive compound (such as a conductive polymer or indium oxide), a metal (such as aluminum, palladium, or gold) or an alloy. Here, the term "conductive" denotes that the volume resistivity is less than 10¹³ Ω·cm.

In a case where the electrophotographic photoreceptor is used in a laser printer, for example, it is preferable that the surface of the conductive substrate is roughened such that a centerline average roughness Ra thereof is 0.04 µm or greater and 0.5 µm or less for the purpose of suppressing interference fringes from occurring in a case of irradiation with laser beams. Further, in a case where incoherent light is used as a light source, roughening of the surface to prevent interference fringes is not particularly necessary, and it is appropriate for longer life because occurrence of defects due to the roughness of the surface of the conductive substrate is suppressed.

Examples of the roughening method include wet honing performed by suspending an abrasive in water and spraying the suspension to the conductive substrate, centerless grinding performed by pressure-welding the conductive substrate against a rotating grindstone and continuously grinding the conductive substrate, and an anodizing treatment.

Examples of the roughening method also include a method of dispersing conductive or semi-conductive powder in a resin without roughening the surface of the conductive substrate to form a layer on the surface of the conductive substrate, and performing roughening using the particles dispersed in the layer.

The roughening treatment performed by anodization is a treatment of forming an oxide film on the surface of the conductive substrate by carrying out anodization in an electrolytic solution using a conductive substrate made of a metal (for example, aluminum) as an anode. Examples of the electrolytic solution include a sulfuric acid solution and an oxalic acid solution. However, a porous anodized film formed by anodization is chemically active in a natural state, is easily contaminated, and has a large resistance fluctuation depending on the environment. Therefore, for example, it is preferable that a sealing treatment is performed on the porous anodized film so that the micropores of the oxide film are closed by volume expansion due to a hydration reaction in pressurized steam or boiling water (a metal salt such as nickel may be added thereto) for a change into a more stable a hydrous oxide.

The film thickness of the anodized film is, for example, preferably 0.3 µm or greater and 15 µm or less. In a case where the film thickness is in the above-described range, the barrier properties against injection tend to be exhibited, and an increase in the residual potential due to repeated use tends to be suppressed.

The conductive substrate may be subjected to a treatment with an acidic treatment liquid or a boehmite treatment.

The treatment with an acidic treatment liquid is carried out, for example, as follows. First, an acidic treatment liquid containing phosphoric acid, chromic acid, and hydrofluoric acid is prepared. In the blending ratio of phosphoric acid, chromic acid, and hydrofluoric acid to the acidic treatment liquid, for example, the concentration of the phosphoric acid is 10% by mass or greater and 11% by mass or less, the concentration of the chromic acid is 3% by mass or greater and 5% by mass or less, and the concentration of the hydrofluoric acid is 0.5% by mass or greater and 2% by mass or less, and the concentration of all these acids may be 13.5% by mass or greater and 18% by mass or less. The treatment temperature is, for example, preferably 42°C or higher and 48°C or lower. The film thickness of the coating film is, for example, preferably 0.3 µm or greater and 15 µm or less.

The boehmite treatment is carried out, for example, by dipping the conductive substrate in pure water at 90°C or higher and 100°C or lower for 5 minutes to 60 minutes or by bringing the conductive substrate into contact with heated steam at 90°C or higher and 120°C or lower for 5 minutes to 60 minutes. The film thickness of the coating film is, for example, preferably 0.1 µm or greater and 5 µm or less. This coating film may be further subjected to the anodizing treatment using an electrolytic solution having low film solubility, such as adipic acid, boric acid, a borate, a phosphate, a phthalate, a maleate, a benzoate, a tartrate, or a citrate.

### [Undercoat Layer]

The undercoat layer is, for example, a layer containing inorganic particles and a binder resin.

Examples of the inorganic particles include inorganic particles having a powder resistance (volume resistivity) of 10² Ω·cm or greater and 10¹¹ Ω·cm or less.

Among these, as the inorganic particles having the above-described resistance value, for example, metal oxide particles such as tin oxide particles, titanium oxide particles, zinc oxide particles, and zirconium oxide particles may be used, and zinc oxide particles are particularly preferable.

The specific surface area of the inorganic particles measured by the BET method may be, for example, 10 m²/g or greater.

The volume average particle diameter of the inorganic particles may be, for example, 50 nm or greater and 2,000 nm or less (for example, preferably 60 nm or greater and 1,000 nm or less).

The content of the inorganic particles is, for example, preferably 10% by mass or greater and 80% by mass or less and more preferably 40% by mass or greater and 80% by mass or less with respect to the amount of the binder resin.

The inorganic particles may be subjected to a surface treatment. As the inorganic particles, inorganic particles subjected to different surface treatments or inorganic particles having different particle diameters may be used in the form of a mixture of two or more kinds thereof.

Examples of the surface treatment agent include a silane coupling agent, a titanate-based coupling agent, an aluminum-based coupling agent, and a surfactant. In particular, for example, a silane coupling agent is preferable, and a silane coupling agent containing an amino group is more preferable.

Examples of the silane coupling agent containing an amino group include 3-aminopropyltriethoxysilane, N-2-(aminoethyl)-3-aminopropyltrimethoxysilane, N-2-(aminoethyl)-3-aminopropylmethyldimethoxysilane, and N,N-bis(2-hydroxyethyl)-3-aminopropyltriethoxysilane, but are not limited thereto.

The silane coupling agent may be used in the form of a mixture of two or more kinds thereof. For example, a silane coupling agent containing an amino group and another silane coupling agent may be used in combination. Examples of other silane coupling agents include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl) -3-aminopropyltriethoxysilane, and 3-chloropropyltrimethoxysilane, but are not limited thereto.

The surface treatment method using a surface treatment agent may be any method as long as the method is a known method, and any of a dry method or a wet method may be used.

The treatment amount of the surface treatment agent is, for example, preferably 0.5% by mass or greater and 10% by mass or less with respect to the amount of the inorganic particles.

Here, the undercoat layer may contain an electron-accepting compound (acceptor compound) together with the inorganic particles, for example, from the viewpoint of enhancing the long-term stability of the electrical properties and the carrier blocking properties.

Examples of the electron-accepting compound include electron-transporting substances, for example, a quinone-based compound such as chloranil or bromanil; a tetracyanoquinodimethane-based compound; a fluorenone compound such as 2,4,7-trinitrofluorenone or 2,4,5,7-tetranitro-9-fluorenone; an oxadiazole-based compound such as 2-(4-biphenyl)-5-(4-t-butylphenyl)-1,3,4-oxadiazole, 2,5-bis(4-naphthyl)-1,3,4-oxadiazole, or 2,5-bis(4-diethylaminophenyl)-1,3,4-oxadiazole; a xanthone-based compound; a thiophene compound; a diphenoquinone compound such as 3,3',5,5'-tetra-t-butyldiphenoquinone; and a benzophenone compound.

In particular, as the electron-accepting compound, for example, a compound having an anthraquinone structure is preferable. As the compound having an anthraquinone structure, for example, a hydroxyanthraquinone compound, an aminoanthraquinone compound, or an aminohydroxyanthraquinone compound is preferable, and specifically, for example, anthraquinone, alizarin, quinizarin, anthrarufin, or purpurin is preferable.

The electron-accepting compound may be contained in the undercoat layer in a state of being dispersed with inorganic particles or in a state of being attached to the surface of each inorganic particle.

Examples of the method of attaching the electron-accepting compound to the surface of the inorganic particle include a dry method and a wet method.

The dry method is, for example, a method of attaching the electron-accepting compound to the surface of each inorganic particle by adding the electron-accepting compound dropwise to inorganic particles directly or by dissolving the electron-accepting compound in an organic solvent while stirring the inorganic particles with a mixer having a large shearing force and spraying the mixture together with dry air or nitrogen gas. The electron-accepting compound may be added dropwise or sprayed, for example, at a temperature lower than or equal to the boiling point of the solvent. After the dropwise addition or the spraying of the electron-accepting compound, the compound may be further baked at 100°C or higher. The baking is not particularly limited as long as the temperature and the time are adjusted such that the electrophotographic characteristics can be obtained.

The wet method is, for example, a method of attaching the electron-accepting compound to the surface of each inorganic particle by adding the electron-accepting compound to inorganic particles while dispersing the inorganic particles in a solvent by performing stirring or using ultrasonic waves, a sand mill, an attritor, or a ball mill, stirring or dispersing the mixture, and removing the solvent. The solvent removing method is carried out by, for example, filtration or distillation so that the solvent is distilled off. After removal of the solvent, the mixture may be further baked at 100°C or higher. The baking is not particularly limited as long as the temperature and the time are adjusted such that the electrophotographic characteristics can be obtained. In the wet method, the moisture contained in the inorganic particles may be removed before the electron-accepting compound is added, and examples thereof include a method of removing the moisture while stirring and heating the moisture in a solvent and a method of removing the moisture by azeotropically boiling the moisture with a solvent.

Further, the electron-accepting compound may be attached to the surface before or after the inorganic particles are subjected to a surface treatment with a surface treatment agent or simultaneously with the surface treatment performed on the inorganic particles with a surface treatment agent.

The content of the electron-accepting compound may be, for example, 0.01% by mass or greater and 20% by mass or less and preferably 0.01% by mass or greater and 10% by mass or less with respect to the amount of the inorganic particles.

Examples of the binder resin used for the undercoat layer include known polymer compounds such as an acetal resin (such as polyvinyl butyral), a polyvinyl alcohol resin, a polyvinyl acetal resin, a casein resin, a polyamide resin, a cellulose resin, gelatin, a polyurethane resin, a polyester resin, an unsaturated polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a urea resin, a phenol resin, a phenol-formaldehyde resin, a melamine resin, a urethane resin, an alkyd resin, and an epoxy resin; a zirconium chelate compound; a titanium chelate compound; an aluminum chelate compound; a titanium alkoxide compound; an organic titanium compound; and known materials such as a silane coupling agent.

Examples of the binder resin used for the undercoat layer include a charge-transporting resin containing a charge-transporting group, and a conductive resin (such as polyaniline).

Among these, as the binder resin used for the undercoat layer, for example, a resin insoluble in a coating solvent of the upper layer is preferable, and a resin obtained by reaction between a curing agent and at least one resin selected from the group consisting of a thermosetting resin such as a urea resin, a phenol resin, a phenol-formaldehyde resin, a melamine resin, a urethane resin, an unsaturated polyester resin, an alkyd resin, or an epoxy resin; a polyamide resin, a polyester resin, a polyether resin, a methacrylic resin, an acrylic resin, a polyvinyl alcohol resin, and a polyvinyl acetal resin is particularly preferable.

In a case where these binder resins are used in combination of two or more kinds thereof, the mixing ratio thereof is set as necessary.

The undercoat layer may contain various additives for improving the electrical properties, the environmental stability, and the image quality.

Examples of the additives include known materials, for example, an electron-transporting pigment such as a polycyclic condensed pigment or an azo-based pigment, a zirconium chelate compound, a titanium chelate compound, an aluminum chelate compound, a titanium alkoxide compound, an organic titanium compound, and a silane coupling agent. The silane coupling agent is used for a surface treatment of the inorganic particles as described above, but may be further added to the undercoat layer as an additive.

Examples of the silane coupling agent serving as an additive include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl)-3-aminopropyltriethoxysilane, and 3-chloropropyltrimethoxysilane.

Examples of the zirconium chelate compound include zirconium butoxide, ethyl zirconium acetoacetate, zirconium triethanolamine, acetylacetonate zirconium butoxide, ethyl zirconium butoxide acetoacetate, zirconium acetate, zirconium oxalate, zirconium lactate, zirconium phosphonate, zirconium octanoate, zirconium naphthenate, zirconium laurate, zirconium stearate, zirconium isostearate, zirconium butoxide methacrylate, stearate zirconium butoxide, and isostearate zirconium butoxide.

Examples of the titanium chelate compound include tetraisopropyl titanate, tetranormal butyl titanate, a butyl titanate dimer, tetra(2-ethylhexyl) titanate, titanium acetylacetonate, polytitanium acetylacetonate, titanium octylene glycolate, titanium lactate ammonium salt, titanium lactate, titanium lactate ethyl ester, titanium triethanol aminate, and polyhydroxy titanium stearate.

Examples of the aluminum chelate compound include aluminum isopropylate, monobutoxyaluminum diisopropylate, aluminum butyrate, diethylacetoacetate aluminum diisopropylate, and aluminum tris(ethylacetoacetate).

These additives may be used alone or in the form of a mixture or a polycondensate of a plurality of compounds.

The undercoat layer may have, for example, a Vickers hardness of 35 or greater.

The surface roughness (ten-point average roughness) of the undercoat layer may be adjusted, for example, to 1/2 from 1/(4n) (n represents a refractive index of an upper layer) of a laser wavelength λ for exposure to be used to suppress moire fringes.

Resin particles or the like may be added to the undercoat layer to adjust the surface roughness. Examples of the resin particles include silicone resin particles and crosslinked polymethyl methacrylate resin particles. Further, the surface of the undercoat layer may be polished to adjust the surface roughness. Examples of the polishing method include buff polishing, a sandblast treatment, wet honing, and a grinding treatment.

The formation of the undercoat layer is not particularly limited, and a known forming method is used. For example, a coating film of a coating solution for forming an undercoat layer in which the above-described components are added to a solvent is formed, and the coating film is dried and, as necessary, heated.

Examples of the solvent for preparing the coating solution for forming an undercoat layer include known organic solvents such as an alcohol-based solvent, an aromatic hydrocarbon solvent, a halogenated hydrocarbon solvent, a ketone-based solvent, a ketone alcohol-based solvent, an ether-based solvent, and an ester-based solvent.

Specific examples of these solvents include typical organic solvents such as methanol, ethanol, n-propanol, iso-propanol, n-butanol, benzyl alcohol, methyl cellosolve, ethyl cellosolve, acetone, methyl ethyl ketone, cyclohexanone, methyl acetate, ethyl acetate, n-butyl acetate, dioxane, tetrahydrofuran, methylene chloride, chloroform, chlorobenzene, and toluene.

Examples of the method of dispersing the inorganic particles in a case of preparing the coating solution for forming an undercoat layer include known methods such as a roll mill, a ball mill, a vibration ball mill, an attritor, a sand mill, a colloid mill, and a paint shaker.

Examples of the method of coating the conductive substrate with the coating solution for forming an undercoat layer include typical coating methods such as a blade coating method, a wire bar coating method, a spray coating method, a dip coating method, a bead coating method, an air knife coating method, and a curtain coating method.

The film thickness of the undercoat layer is set to be, for example, preferably in a range of 15 µm or greater and more preferably in a range of 20 µm or greater and 50 µm or less.

### [Interlayer]

Although not shown in the figures, an interlayer may be further provided between the undercoat layer and the photosensitive layer.

The interlayer is, for example, a layer containing a resin. Examples of the resin used for the interlayer include a polymer compound, for example, an acetal resin (such as polyvinyl butyral), a polyvinyl alcohol resin, a polyvinyl acetal resin, a casein resin, a polyamide resin, a cellulose resin, gelatin, a polyurethane resin, a polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a phenol-formaldehyde resin, or a melamine resin.

The interlayer may be a layer containing an organometallic compound. Examples of the organometallic compound used for the interlayer include an organometallic compound containing metal atoms such as zirconium, titanium, aluminum, manganese, and silicon.

The compounds used for the interlayer may be used alone or in the form of a mixture or a polycondensate of a plurality of compounds.

Among these, it is preferable that the interlayer is, for example, a layer containing an organometallic compound having a zirconium atom or a silicon atom.

The formation of the interlayer is not particularly limited, and a known forming method is used. For example, a coating film of a coating solution for forming an interlayer in which the above-described components are added to a solvent is formed, and the coating film is dried and, as necessary, heated.

Examples of the coating method of forming the interlayer include typical methods such as a dip coating method, a push-up coating method, a wire bar coating method, a spray coating method, a blade coating method, an air knife coating method, and a curtain coating method.

The film thickness of the interlayer is set to be, for example, preferably in a range of 0.1 µm or greater and 3 µm or less. Further, the interlayer may be used as the undercoat layer.

### [Charge Generation Layer]

The charge generation layer is, for example, a layer containing a charge generation material and a binder resin. Further, the charge generation layer may be a deposition layer of the charge generation material. The deposition layer of the charge generation material is, for example, preferable in a case where an incoherent light source such as a light emitting diode (LED) or an organic electro-luminescence (EL) image array is used.

Examples of the charge generation material include an azo pigment such as bisazo or trisazo; a fused ring aromatic pigment such as dibromoanthanthrone; a perylene pigment; a pyrrolopyrrole pigment; a phthalocyanine pigment; zinc oxide; and trigonal selenium.

Among these, for example, a metal phthalocyanine pigment or a metal-free phthalocyanine pigment is preferably used as the charge generation material in order to deal with laser exposure in a near infrared region. Specifically, for example, hydroxygallium phthalocyanine; chlorogallium phthalocyanine; dichlorotin phthalocyanine; and titanyl phthalocyanine are more preferable.

On the other hand, for example, a fused ring aromatic pigment such as dibromoanthanthrone; a thioindigo-based pigment; a porphyrazine compound; zinc oxide; trigonal selenium; or a bisazo pigment is preferable as the charge generation material in order to deal with laser exposure in a near ultraviolet region.

The above-described charge generation material may also be used even in a case where an incoherent light source such as an LED or an organic EL image array having a center wavelength of light emission at 450 nm or greater and 780 nm or less is used.

Meanwhile, in a case where an n-type semiconductor such as a fused ring aromatic pigment, a perylene pigment, or an azo pigment is used as the charge generation material, a dark current is unlikely to be generated, and image defects referred to as black spots can be suppressed even in a case where a thin film is used as the photosensitive layer.

Further, the n-type is determined by the polarity of the flowing photocurrent using a typically used time-of-flight method, and a material in which electrons more easily flow as carriers than positive holes is determined as the n-type.

The binder resin used for the charge generation layer is selected from a wide range of insulating resins, and the binder resin may be selected from organic photoconductive polymers such as poly-N-vinylcarbazole, polyvinyl anthracene, polyvinylpyrene, and polysilane.

Examples of the binder resin include a polyvinyl butyral resin, a polyarylate resin (a polycondensate of bisphenols and aromatic divalent carboxylic acid), a polycarbonate resin, a polyester resin, a phenoxy resin, a vinyl chloride-vinyl acetate copolymer, a polyamide resin, an acrylic resin, a polyacrylamide resin, a polyvinylpyridine resin, a cellulose resin, a urethane resin, an epoxy resin, casein, a polyvinyl alcohol resin, and a polyvinylpyrrolidone resin. Here, the term "insulating" denotes that the volume resistivity is 10¹³ Ω·cm or greater.

These binder resins may be used alone or in the form of a mixture of two or more kinds thereof.

Further, the blending ratio between the charge generation material and the binder resin is, for example, preferably in a range of 10:1 to 1:10 in terms of the mass ratio.

The charge generation layer may also contain other known additives.

The formation of the charge generation layer is not particularly limited, and a known forming method is used. For example, a coating film of a coating solution for forming a charge generation layer in which the above-described components are added to a solvent is formed, and the coating film is dried and, as necessary, heated. Further, the charge generation layer may be formed by vapor deposition of the charge generation material. The formation of the charge generation layer by vapor deposition is, for example, particularly appropriate in a case where a fused ring aromatic pigment or a perylene pigment is used as the charge generation material.

Examples of the solvent for preparing the coating solution for forming a charge generation layer include methanol, ethanol, n-propanol, n-butanol, benzyl alcohol, methyl cellosolve, ethyl cellosolve, acetone, methyl ethyl ketone, cyclohexanone, methyl acetate, n-butyl acetate, dioxane, tetrahydrofuran, methylene chloride, chloroform, chlorobenzene, and toluene. These solvents are used alone or in the form of a mixture of two or more kinds thereof.

As a method of dispersing particles (for example, the charge generation material) in the coating solution for forming a charge generation layer, for example, a media disperser such as a ball mill, a vibration ball mill, an attritor, a sand mill, or a horizontal sand mill, or a medialess disperser such as a stirrer, an ultrasonic disperser, a roll mill, or a high-pressure homogenizer is used. Examples of the high-pressure homogenizer include a collision type high-pressure homogenizer in which a dispersion liquid is dispersed by a liquid-liquid collision or a liquid-wall collision in a high-pressure state, and a penetration type high-pressure homogenizer in which a dispersion liquid is dispersed by causing the liquid to penetrate through a micro-flow path in a high-pressure state.

During the dispersion, it is effective to set the average particle diameter of the charge generation material in the coating solution for forming a charge generation layer to 0.5 µm or less, for example, preferably 0.3 µm or less, and more preferably 0.15 µm or less.

Examples of the method of coating the undercoat layer (or the interlayer) with the coating solution for forming a charge generation layer include typical methods such as a blade coating method, a wire bar coating method, a spray coating method, a dip coating method, a bead coating method, an air knife coating method, and a curtain coating method.

The film thickness of the charge generation layer is set to be, for example, preferably in a range of 0.1 µm or greater and 5.0 µm or less and more preferably in a range of 0.2 µm or greater and 2.0 µm or less.

### [Charge Transport Layer]

The charge transport layer is a layer containing a charge transport material and a binder resin. The charge transport layer may be a layer containing a polymer charge transport material.

Examples of the charge transport material include a quinone-based compound such as p-benzoquinone, chloranil, bromanil, or anthraquinone; a tetracyanoquinodimethane-based compound; a fluorenone compound such as 2,4,7-trinitrofluorenone; a xanthone-based compound; a benzophenone-based compound; a cyanovinyl-based compound; and an electron-transporting compound such as an ethylene-based compound. Examples of the charge transport material include a positive hole-transporting compound such as a triarylamine-based compound, a benzidine-based compound, an arylalkane-based compound, an aryl-substituted ethylene-based compound, a stilbene-based compound, an anthracene-based compound, or a hydrazone-based compound. These charge transport materials may be used alone or in combination of two or more kinds thereof, but are not limited thereto.

From the viewpoint of the charge mobility, for example, a triarylamine derivative represented by Structural Formula (a-1) or a benzidine derivative represented by Structural Formula (a-2) is preferable as the charge transport material.

**In** Structural Formula (a-1), Ar^{T1}, Ar^{T2}, and Ar^{T3} each independently represent a substituted or unsubstituted aryl group, -C₆H₄-C(R^{T4})=C(R^{T5})(R^{T6}), or -C₆H₄-CH=CH-CH=C(R^{T7})(R^{T8}). R^{T4}, R^{T5}, R^{T6}, R^{T7}, and R^{T8} each independently represent a hydrogen atom, a substituted or unsubstituted alkyl group, or a substituted or unsubstituted aryl group.

Examples of the substituent of each group described above include a halogen atom, an alkyl group having 1 or more and 5 or less carbon atoms, and an alkoxy group having 1 or more and 5 or less carbon atoms. Further, examples of the substituent of each group described above include a substituted amino group substituted with an alkyl group having 1 or more and 3 or less carbon atoms.

In Structural Formula (a-2), R^{T91} and R^{T92} each independently represent a hydrogen atom, a halogen atom, an alkyl group having 1 or more and 5 or less carbon atoms, or an alkoxy group having 1 or more and 5 or less carbon atoms. R^{T101}, R^{T102}, R^{T111}, and R^{T112} each independently represent a halogen atom, an alkyl group having 1 or more and 5 or less carbon atoms, an alkoxy group having 1 or more and 5 or less carbon atoms, a substituted amino group substituted with an alkyl group having 1 or more and 2 or less carbon atoms, a substituted or unsubstituted aryl group, -C(R^{T12})-C(R^{T13})(R^{T14}), or -CH=CH-CH=C(R^{T15})(R^{T16}), and R^{T12}, R^{T13}, R^{T14}, R^{T15}, and R^{T16} each independently represent a hydrogen atom, a substituted or unsubstituted alkyl group, or a substituted or unsubstituted aryl group. Tm1, Tm2, Tn1, and Tn2 each independently represent an integer of 0 or greater and 2 or less.

Examples of the substituent of each group described above include a halogen atom, an alkyl group having 1 or more and 5 or less carbon atoms, and an alkoxy group having 1 or more and 5 or less carbon atoms. Further, examples of the substituent of each group described above include a substituted amino group substituted with an alkyl group having 1 or more and 3 or less carbon atoms.

Here, among the triarylamine derivative represented by Structural Formula (a-1) and the benzidine derivative represented by Structural Formula (a-2), for example, a triarylamine derivative having "-C₆H₄-CH=CH-CH=C(R^{T7})(R^{T8})" and a benzidine derivative having "-CH=CH-CH=C(R^{T15})(R^{T16})" are particularly preferable from the viewpoint of the charge mobility.

As the polymer charge transport material, known materials having charge transport properties, such as poly-N-vinylcarbazole and polysilane, can be used. Particularly, for example, a polyester-based polymer charge transport material is particularly preferable. Further, the polymer charge transport material may be used alone or in combination of binder resins.

As the binder resin used in the charge transport layer, the charge transport layer may contain other resins in addition to the polyester resin P_{A} and the polycarbonate resin P_{B} described above within a range where the effects of the abrasion resistance and the property of suppressing abnormal discharge are not impaired.

Examples of other resins include a polycarbonate resin other than the polycarbonate resin P_{B}, a polyester resin other than the polyester resin P_{A}, a polyarylate resin, a methacrylic resin, an acrylic resin, a polyvinyl chloride resin, a polyvinylidene chloride resin, a polystyrene resin, a polyvinyl acetate resin, a styrene-butadiene copolymer, a vinylidene chloride-acrylonitrile copolymer, a vinyl chloride-vinyl acetate copolymer, a vinyl chloride-vinyl acetate-maleic anhydride copolymer, a silicone resin, a silicone alkyd resin, a phenol-formaldehyde resin, a styrene-alkyd resin, poly-N-vinylcarbazole, and polysilane. Among these, for example, a polycarbonate resin or a polyarylate resin is preferable as the binder resin. Such other resins may be used alone or in combination of two or more kinds thereof.

Further, the blending ratio between the charge transport material and the binder resin is, for example, preferably in a range of 10:1 to 1:5 in terms of the mass ratio.

The charge transport layer may also contain other known additives.

The formation of the charge transport layer is not particularly limited, and a known forming method is used. For example, a coating film of a coating solution for forming a charge transport layer in which the above-described components are added to a solvent is formed, and the coating film is dried and, as necessary, heated.

Examples of the solvent for preparing the coating solution for forming a charge transport layer include typical organic solvents, for example, aromatic hydrocarbons such as benzene, toluene, xylene, and chlorobenzene; ketones such as acetone and 2-butanone; halogenated aliphatic hydrocarbons such as methylene chloride, chloroform, and ethylene chloride; and cyclic or linear ethers such as tetrahydrofuran and ethyl ether. These solvents are used alone or in the form of a mixture of two or more kinds thereof.

Examples of the coating method of coating the charge generation layer with the coating solution for forming a charge transport layer include typical methods such as a blade coating method, a wire bar coating method, a spray coating method, a dip coating method, a bead coating method, an air knife coating method, and a curtain coating method.

The film thickness of the charge transport layer is set to be, for example, preferably in a range of 5 µm or greater and 50 µm or less and more preferably in a range of 10 µm or greater and 30 µm or less.

### [Single Layer Type Photosensitive Layer]

The single layer type photosensitive layer (charge generation layer/charge transport layer) is, for example, a layer containing a charge generation material, a charge transport material, a binder resin, and as necessary, other known additives. Further, these materials are the same as the materials described in the sections of the outermost layer, the charge generation layer, and the charge transport layer.

Further, the content of the charge generation material in the single layer type photosensitive layer may be, for example, 0.1% by mass or greater and 10% by mass or less and preferably 0.8% by mass or greater and 5% by mass or less with respect to the total solid content.

Further, the content of the charge transport material in the single layer type photosensitive layer may be, for example, 5% by mass or greater and 50% by mass or less with respect to the total solid content.

The method of forming the single layer type photosensitive layer is the same as the method of forming the charge generation layer or the charge transport layer.

The film thickness of the single layer type photosensitive layer may be, for example, 5 µm or greater and 50 µm or less and preferably 10 µm or greater and 40 µm or less.

### <Image Forming Apparatus (And Process Cartridge)>

An image forming apparatus according to the present exemplary embodiment includes the electrophotographic photoreceptor, a charging device that charges a surface of the electrophotographic photoreceptor, an electrostatic latent image forming device that forms an electrostatic latent image on the charged surface of the electrophotographic photoreceptor, a developing device that develops the electrostatic latent image formed on the surface of the electrophotographic photoreceptor with a developer containing a toner to form a toner image, and a transfer device that transfers the toner image to a surface of a recording medium. Further, the electrophotographic photoreceptor according to the present exemplary embodiment is employed as the electrophotographic photoreceptor, and the charging device that comes into direct contact with the surface of the electrophotographic photoreceptor and applies only a DC voltage to charge the surface of the electrophotographic photoreceptor is employed as the charging device.

Further, in the image forming apparatus according to the present exemplary embodiment, for example, an aspect in which the charging device includes a charging member that charges the surface of the electrophotographic photoreceptor and a DC voltage application unit that applies only the DC voltage to the charging member, and the voltage applied to the charging member from the DC voltage application unit is -700 V or greater and -300 V or less (for example, more preferably -650 V or greater and -450 V or less) is preferable.

The abnormal discharge can be effectively suppressed even under such charging conditions.

As the image forming apparatus according to the present exemplary embodiment, known image forming apparatuses such as an apparatus including a fixing device that fixes a toner image transferred to the surface of a recording medium; a direct transfer type apparatus that transfers a toner image formed on the surface of an electrophotographic photoreceptor directly to a recording medium; an intermediate transfer type apparatus that primarily transfers a toner image formed on the surface of an electrophotographic photoreceptor to the surface of an intermediate transfer member and secondarily transfers the toner image transferred to the surface of the intermediate transfer member to the surface of a recording medium; an apparatus including a cleaning device that cleans the surface of an electrophotographic photoreceptor after the transfer of a toner image and before the charging; an apparatus including a charge erasing device that erases the charges on the surface of an electrophotographic photoreceptor by applying the charge erasing light after the transfer of a toner image and before the charging; and an apparatus including an electrophotographic photoreceptor heating member for increasing the temperature of an electrophotographic photoreceptor and decreasing the relative temperature are employed.

**In** a case of the intermediate transfer type apparatus, the transfer device is, for example, configured to include an intermediate transfer member having a surface onto which the toner image is transferred, a primary transfer device primarily transferring the toner image formed on the surface of the electrophotographic photoreceptor to the surface of the intermediate transfer member, and a secondary transfer device secondarily transferring the toner image transferred to the surface of the intermediate transfer member to the surface of the recording medium.

The image forming apparatus according to the present exemplary embodiment may be any of a dry development type image forming apparatus or a wet development type (development type using a liquid developer) image forming apparatus.

Further, in the image forming apparatus according to the present exemplary embodiment, for example, the portion including the electrophotographic photoreceptor may have a cartridge structure (process cartridge) that is attachable to and detachable from the image forming apparatus. As the process cartridge, for example, a process cartridge including the electrophotographic photoreceptor according to the present exemplary embodiment is preferably used. Further, the process cartridge may include, for example, at least one selected from the group consisting of a charging device, an electrostatic latent image forming device, a developing device, and a transfer device in addition to the electrophotographic photoreceptor.

Hereinafter, an example of the image forming apparatus according to the present exemplary embodiment will be described, but the present exemplary embodiment is not limited thereto. Further, main parts shown in the figures will be described, but description of other parts will not be provided.

Fig. 3 is a schematic configuration view showing an example of an image forming apparatus according to the present exemplary embodiment.

As shown in Fig. 3, an image forming apparatus 100 according to the present exemplary embodiment includes a process cartridge 300 including an electrophotographic photoreceptor 7, an exposure device 9 (an example of an electrostatic latent image forming device), a transfer device 40 (primary transfer device), and an intermediate transfer member 50. Further, in the image forming apparatus 100, the exposure device 9 is disposed at a position that can be exposed to the electrophotographic photoreceptor 7 from an opening portion of the process cartridge 300, the transfer device 40 is disposed at a position that faces the electrophotographic photoreceptor 7 via the intermediate transfer member 50, and the intermediate transfer member 50 is disposed such that a part of the intermediate transfer member 50 is in contact with the electrophotographic photoreceptor 7. Although not shown, the image forming apparatus also includes a secondary transfer device that transfers the toner image transferred to the intermediate transfer member 50 to a recording medium (for example, paper). Further, the intermediate transfer member 50, the transfer device 40 (primary transfer device), and the secondary transfer device (not shown) correspond to an example of the transfer device.

The process cartridge 300 in Fig. 3 integrally supports the electrophotographic photoreceptor 7, a charging device 8 (an example of the charging device), a developing device 11 (an example of the developing device), and a cleaning device 13 (an example of the cleaning device) in a housing. The cleaning device 13 has a cleaning blade (an example of the cleaning member) 131, and the cleaning blade 131 is disposed to come into contact with the surface of the electrophotographic photoreceptor 7. Further, the cleaning member may be a conductive or insulating fibrous member instead of the aspect of the cleaning blade 131, and may be used alone or in combination with the cleaning blade 131.

Further, Fig. 3 shows an example of an image forming apparatus including a fibrous member 132 (roll shape) that supplies a lubricant 14 to the surface of the electrophotographic photoreceptor 7 and a fibrous member 133 (flat brush shape) that assists cleaning, but these are disposed as necessary.

Hereinafter, each configuration of the image forming apparatus according to the present exemplary embodiment will be described.

### - Charging Device -

It is preferable that the charging device 8 includes, for example, a charging member that is provided in contact with the surface of the photoreceptor and charges the surface of the photoreceptor, and a power source (an example of a voltage application unit) that applies a charging voltage to the charging member. As described above, it is preferable that the power source is, for example, a DC voltage application unit that applies only a DC voltage to the charging member. Further, the voltage to be applied to the charging member from the power source that is the DC voltage application unit is, for example, preferably -700 V or greater and -300 V or less (for example, more preferably -650 V or greater and -450 V or less).

Examples of the charging member of the charging device 8 include a contact type charger using a conductive charging roller, a charging brush, a charging film, a charging rubber blade, a charging tube, or the like.

### - Exposure Device -

Examples of the exposure device 9 include an optical system device that exposes the surface of the electrophotographic photoreceptor 7 to light such as a semiconductor laser beam, LED light, and liquid crystal shutter light in a predetermined image pattern. The wavelength of the light source is within the spectral sensitivity region of the electrophotographic photoreceptor. As the wavelength of a semiconductor laser, near infrared, which has an oscillation wavelength in the vicinity of 780 nm, is mostly used. However, the wavelength is not limited thereto, and a laser having an oscillation wavelength of an approximately 600 nm level or a laser having an oscillation wavelength of 400 nm or greater and 450 nm or less as a blue laser may also be used. Further, a surface emission type laser light source capable of outputting a multi-beam is also effective for forming a color image.

### - Developing Device -

Examples of the developing device 11 include a typical developing device that performs development in contact or non-contact with the developer. The developing device 11 is not particularly limited as long as the developing device has the above-described functions, and is selected depending on the purpose thereof. Examples of the developing device include known developing machines having a function of attaching a one-component developer or a two-component developer to the electrophotographic photoreceptor 7 using a brush, a roller, or the like. Among these, for example, a developing device formed of a developing roller having a surface on which a developer is held is preferably used.

The developer used in the developing device 11 may be a one-component developer containing only a toner or a two-component developer containing a toner and a carrier. Further, the developer may be magnetic or non-magnetic. Known developers are employed as these developers.

### - Cleaning Device -

As the cleaning device 13, a cleaning blade type device including the cleaning blade 131 is used.

In addition to the cleaning blade type device, a fur brush cleaning type device or a simultaneous development cleaning type device may be employed.

### - Transfer Device -

Examples of the transfer device 40 include a known transfer charger such as a contact type transfer charger using a belt, a roller, a film, a rubber blade or the like, or a scorotron transfer charger or a corotron transfer charger using corona discharge.

### - Intermediate Transfer Member -

As the intermediate transfer member 50, a belt-like intermediate transfer member (intermediate transfer belt) containing semi-conductive polyimide, polyamide-imide, polycarbonate, polyarylate, polyester, rubber, or the like is used. Further, as the form of the intermediate transfer member, a drum-like intermediate transfer member may be used in addition to the belt-like intermediate transfer member.

Fig. 4 is a schematic configuration view showing an example of an image forming apparatus according to the present exemplary embodiment.

An image forming apparatus 120 shown in Fig. 4 is a tandem type multicolor image forming apparatus on which four process cartridges 300 are mounted. The image forming apparatus 120 is formed such that four process cartridges 300 are arranged in parallel on the intermediate transfer member 50, and one electrophotographic photoreceptor is used for each color. Further, the image forming apparatus 120 has the same configuration as the image forming apparatus 100 except that the image forming apparatus 120 is of a tandem type.

### Examples

Hereinafter, exemplary embodiments of the invention will be described in detail based on examples, but the exemplary embodiments of the invention are not limited to the examples. In the following description, "parts" and "%" are on a mass basis unless otherwise specified.

In the following description, the synthesis, the treatment, and the production are carried out at room temperature (25°C ± 3°C) unless otherwise specified.

### <Preparation of Polyester Resin>

· A polyester resin 1 (PE1) having 50% by mole of a dicarboxylic acid unit (A2-3) and 50% by mole of a diol unit (B1-3) is prepared.
· A polyester resin 2 (PE2) having 50% by mole of a dicarboxylic acid unit (A2-3) and 50% by mole of a diol unit (B1-4) is prepared.
· A polyester resin 3 (PE3) having 25% by mole of a dicarboxylic acid unit (A2-3), 25% by mole of a dicarboxylic acid unit (A4-3), and 50% by mole of a diol unit (B4-4) is prepared.
· A polyester resin 4 (PE4) having 50% by mole of a dicarboxylic acid unit (A3-1) and 50% by mole of a diol unit (B4-3) is prepared.

### <Preparation of Polycarbonate Resin>

· A polycarbonate resin 1 (PC1) having the following structure is prepared. A molar ratio m:n in PC1 is 25:75, and the weight-average molecular weight of the polycarbonate resin is 50,000.
· A polycarbonate resin 2 (PC2) having the following structure is prepared. The weight-average molecular weight of PC2 is 50,000.
· A polycarbonate resin 3 (PC3) having the following structure is prepared. A molar ratio m:n in PC3 is 15:85, and the weight-average molecular weight of PC3 is 40,000.

The elastic deformation rate of the resin is determined by the method described above.

The results are listed in Table 1.

### <Production of Electrophotographic Photoreceptor Including Lamination Type Photosensitive Layer>

### [Electrophotographic Photoreceptor (P1)]

### - Formation of Undercoat Layer -

A cylindrical aluminum tube having an outer diameter of 30 mm, a length of 250 mm, and a thickness of 1 mm is prepared as a conductive substrate.

100 parts of zinc oxide (average particle diameter of 70 nm, specific surface area of 15 m²/g, manufactured by Tayca Corporation) is stirred and mixed with 500 parts of toluene, 1.3 parts of a silane coupling agent (trade name: KBM-603, manufactured by Shin-Etsu Chemical Co., Ltd., N-2-(aminoethyl)-3-aminopropyltrimethoxysilane) is added thereto, and the mixture is stirred for 2 hours. Thereafter, toluene is distilled off under reduced pressure and baked at 120°C for 3 hours to obtain zinc oxide subjected to a surface treatment with a silane coupling agent.

110 parts of the surface-treated zinc oxide is stirred and mixed with 500 parts of tetrahydrofuran, a solution obtained by dissolving 0.6 parts of alizarin in 50 parts of tetrahydrofuran is added thereto, and the mixture is stirred at 50°C for 5 hours. Thereafter, the solid content is separated by filtration by carrying out filtration under reduced pressure and dried at 60°C under reduced pressure, thereby obtaining zinc oxide with alizarin.

100 parts of a solution obtained by dissolving 60 parts of the zinc oxide with alizarin, 13.5 parts of a curing agent (blocked isocyanate, trade name: SUMIDUR 3175, manufactured by Sumika Covestro Urethane Company, Ltd.), and 15 parts of a butyral resin (trade name: S-LEC BM-1, manufactured by Sekisui Chemical Co., Ltd.) in 68 parts of methyl ethyl ketone is mixed with 5 parts of methyl ethyl ketone, and the solution is dispersed in a sand mill for 2 hours using 1 mmφ glass beads, thereby obtaining a dispersion liquid. 0.005 parts of dioctyltin dilaurate as a catalyst and 4 parts of silicone resin particles (trade name: TOSPEARL 145, manufactured by Momentive Performance Materials Inc.) are added to the dispersion liquid, thereby obtaining a coating solution for forming an undercoat layer. The outer peripheral surface of the conductive substrate is coated with the coating solution for forming an undercoat layer by a dip coating method, and dried and cured at 170°C for 40 minutes to form an undercoat layer with an average thickness of 24 µm.

### - Formation of Charge Generation Layer -

A mixture of 15 parts of hydroxygallium phthalocyanine as a charge generation material (having diffraction peaks at positions where Bragg angles (2θ ± 0.2°) in the X-ray diffraction spectrum using Cukα characteristic X-rays are at least of 7.5°, 9.9°, 12.5, 16.3°, 18.6°, 25.1°, and 28.3°), 10 parts of a vinyl chloride-vinyl acetate copolymer resin (trade name: VMCH, Nippon Unicar Company Limited) as a binder resin, and 200 parts of n-butyl acetate is dispersed in a sand mill for 4 hours using glass beads having a diameter of 1 mm. 175 parts of n-butyl acetate and 180 parts of methyl ethyl ketone are added to the dispersion liquid, and the mixture is stirred, thereby obtaining a coating solution for forming a charge generation layer. The undercoat layer is dipped in and coated with the coating solution for forming a charge generation layer, and dried at room temperature (25°C ± 3°C) to form a charge generation layer having an average thickness of 0.18 µm.

### - Formation of Charge Transport Layer -

45 parts of a benzidine compound represented by Formula (CTM1) as a charge transport material, 49.5 parts of the resin 1 (polyester resin 1 (PE1)) as a binder resin, 5.5 parts of the resin 2 (polycarbonate resin 1 (PC1)) as a binder resin are dissolved in 350 parts of toluene and 150 parts of tetrahydrofuran and treated with a high-pressure homogenizer 5 times, thereby preparing a coating solution for a charge transport layer.

The charge generation layer is coated with the obtained coating solution by a dip coating method and heated at 130°C for 45 minutes, thereby forming a charge transport layer having a film thickness of 31 µm.

### [Electrophotographic Photoreceptors (P2) to (P15) and (CP1) to (CP4)]

Each electrophotographic photoreceptor is prepared in the same manner as in the preparation of the electrophotographic photoreceptor (P1) except that the kinds of the binder resins and the ratio (mass basis) between the amounts of the binder resins are changed as in Table 1 in the formation of the charge transport layer.

### <Preparation of Image Forming Apparatus>

Each electrophotographic photoreceptor obtained as described above is attached to Apeos C2060 (manufactured by FUJIFILM Business Innovation Corporation) to obtain an image forming apparatus of each example.

Further, in the charging device of the image forming apparatus of each example in the following evaluation, the voltage application unit applies only the DC voltage to the charging member, and the voltage (also referred to as "applied voltage") applied from the voltage application unit to the charging member is set to -600 V.

### <Evaluation of Abrasion Resistance>

First, the film thickness of the photosensitive layer is measured, and the measured value is defined as L1.

The image forming apparatus of each example is used to continuously perform printing on 10,000 sheets using a random text chart with an image density of 5% in an environment of a temperature of 20°C and a humidity of 40% RH, the photoreceptor is taken out, the film thickness of the photosensitive layer is measured again, and the measured value is defined as L2. Next, an absolute value of a difference ΔL between L1 and L2 is calculated.

Further, the film thickness is measured using an eddy current film thickness meter. The evaluation standards are as follows.
A: ΔL is 2.0 µm or less
B: ΔL is greater than 2.0 µm and 5.0 µm or less
C: ΔL is greater than 5.0 µm

### <Evaluation of Abnormal Discharge>

The image forming apparatus of each example is used to continuously perform printing on 5,000 sheets of A4 paper using a random text chart with an image density of 5% in a high-temperature and high-humidity environment of 28°C and 85% RH. Thereafter, a 20% halftone image is output, the number of minute color lines on the image is counted, and abnormal discharge is evaluated according to the following standards. It can be said that the abnormal discharge decreases as the number of minute color lines on the image decreases.
A: Abnormal discharge is not found
B: The number of color lines is 1 or greater and 5 or less
D: The number of color lines is 6 or greater

### <Evaluation of Cleaning Properties>

10,000 sheets of random charts with an image density of 1% are output using the image forming apparatus of each example, and one sheet of an A3-sized image with an image density of 100% is output. Immediately after the output of the A3-sized image, streaks due to the residues remaining on the surface of the photoreceptor in the modified machine are observed, the number of streaks is counted, and the cleaning properties are evaluated according to the following standards.
A: Streaks are not found
B: The number of streaks is 5 or less
D: A plurality of (6 or more) streaks occur on the entire surface

**[Table 1]**

| | Photoreceptor No. | Resin 1 | | Resin 2 | | Physical properties | | Evaluation | | |
|---|---|---|---|---|---|---|---|---|---|---|
| | | Type | Elastic deformation rate [%] | Type | Elastic deformation rate [%] | Difference in elastic deformation rate [%] | Ratio between resins [resin 1:resin 2] | Abrasion | Abnormal discharge | Cleaning properties |
| Example 1 | (P1) | PE1 | 58.0 | PC1 | 48.0 | 10.0 | 9:1 | A | B | B |
| Example 2 | (P2) | PE1 | 58.0 | PC1 | 48.0 | 10.0 | 7:3 | A | A | A |
| Example 3 | (P3) | PE1 | 58.0 | PC1 | 48.0 | 10.0 | 5:5 | A | A | A |
| Example 4 | (P4) | PE1 | 58.0 | PC1 | 48.0 | 10.0 | 3:7 | B | A | A |
| Example 5 | (P5) | PE1 | 58.0 | PC1 | 48.0 | 10.0 | 1:9 | B | B | B |
| Example 6 | (P6) | PE2 | 53.8 | PC1 | 48.0 | 5.8 | 9:1 | A | B | B |
| Example 7 | (P7) | PE2 | 53.8 | PC1 | 48.0 | 5.8 | 7:3 | B | B | B |
| Example 8 | (P8) | PE2 | 53.8 | PC1 | 48.0 | 5.8 | 5:5 | B | A | A |
| Example 9 | (P9) | PE2 | 53.8 | PC1 | 48.0 | 5.8 | 3:7 | B | B | B |
| Example 10 | (P10) | PE2 | 53.8 | PC1 | 48.0 | 5.8 | 1:9 | B | B | B |
| Example 11 | (P11) | PE3 | 59.4 | PC1 | 48.0 | 11.4 | 9:1 | A | A | B |
| Example 12 | (P12) | PE3 | 59.4 | PC1 | 48.0 | 11.4 | 7:3 | A | A | A |
| Example 13 | (P13) | PE3 | 59.4 | PC1 | 48.0 | 11.4 | 5:5 | A | A | A |
| Example 14 | (P14) | PE3 | 59.4 | PC1 | 48.0 | 11.4 | 3:7 | B | A | A |
| Example 15 | (P15) | PE3 | 59.4 | PC1 | 48.0 | 11.4 | 1:9 | B | A | B |
| Comparative Example 1 | (CP1) | PE1 | 58.0 | PC2 | 44.0 | 14.0 | 7:3 | A | C | C |
| Comparative Example 2 | (CP2) | PE1 | 58.0 | PC3 | 45.2 | 12.8 | 7:3 | A | C | C |
| Comparative Example 3 | (CP3) | PE4 | 48.5 | PC1 | 48.0 | 0.5 | 7:3 | C | C | C |
| Comparative Example 4 | (CP4) | PE1 | 58.0 | - | - | - | - | A | C | C |

As listed in the table, it has been found that the electrophotographic photoreceptors of the examples are excellent in the abrasion resistance, the property of suppressing a local abnormal discharge phenomenon, and the cleaning properties as compared with the electrophotographic photoreceptors of the comparative examples.

The present exemplary embodiment includes the following aspects.
(((1))) An electrophotographic photoreceptor comprising:
   an outermost layer that contains a charge transport material and a binder resin,
   wherein the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by a range of 5% or greater and 12% or less.
(((2))) The electrophotographic photoreceptor according to (((1))),
   wherein a content ratio (polyester resin Pa:Polycarbonate resin P_{B}) of the polyester resin P_{A} to the polycarbonate resin P_{B} is in a range of 7:3 to 3:7 in terms of a mass.
(((3))) The electrophotographic photoreceptor according to (((2))),
   wherein the content ratio (polyester resin P_{A}:Polycarbonate resin P_{B}) of the polyester resin P_{A} to the polycarbonate resin P_{B} is in a range of 7:3 to 5:5 in terms of the mass.
(((4))) The electrophotographic photoreceptor according to any one of (((1))) to (((3))), wherein the polyester resin P_{A} includes a polyester resin having a dicarboxylic acid unit (A) represented by Formula (A) and a diol unit (B) represented by Formula (B).
(((5))) The electrophotographic photoreceptor according to any one of (((1))) to (((4))), wherein the polycarbonate resin P_{B} includes a polycarbonate resin having a constitutional unit represented by Formula (PCA) and a constitutional unit represented by Formula (PCB).
(((6))) A process cartridge comprising:
   the electrophotographic photoreceptor according to any one of (((1))) to (((5))),
   wherein the process cartridge is attachable to and detachable from an image forming apparatus.
(((7))) An image forming apparatus comprising:
   the electrophotographic photoreceptor according to any one of (((1))) to (((5)));
   a charging device that comes into direct contact with a surface of the electrophotographic photoreceptor and applies only a DC voltage to charge the surface of the electrophotographic photoreceptor;
   an electrostatic latent image forming device that forms an electrostatic latent image on the charged surface of the electrophotographic photoreceptor;
   a developing device that develops the electrostatic latent image formed on the surface of the electrophotographic photoreceptor with a developer containing a toner to form a toner image; and
   a transfer device that transfers the toner image to a surface of a recording medium.
(((8))) The image forming apparatus according to (((7))),
   wherein the charging device includes a charging member that charges the surface of the electrophotographic photoreceptor and a DC voltage application unit that applies only the DC voltage to the charging member, and
   a voltage applied to the charging member from the DC voltage application unit is -700 V or greater and -300 V or less.

According to (((1))), (((4))), or (((5))), it is possible to provide an electrophotographic photoreceptor that has excellent abrasion resistance and is capable of suppressing abnormal discharge even in a case of being charged with only a DC voltage as compared with a case where the electrophotographic photoreceptor has an outermost layer containing a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by less than 5% or greater than 12%.

According to (((2))) or (((3))), it is possible to provide an electrophotographic photoreceptor that has excellent abrasion resistance and is capable of suppressing abnormal discharge even in a case of being charged with only a DC voltage as compared with a case where polyester resin P_{A}:polycarbonate resin P_{B} is out of the range of 7:3 to 3:7 in terms of the mass.

According to (((6))), (((7))), or (((8))), it is possible to provide a process cartridge or an image forming apparatus, including an electrophotographic photoreceptor that has excellent abrasion resistance and is capable of suppressing abnormal discharge even in a case of being charged with only a DC voltage as compared with a case where the electrophotographic photoreceptor has an outermost layer containing a charge transport material and a binder resin, and the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by less than 5% or greater than 12%.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated.

### Brief Description of the Reference Symbols

1: conductive substrate
2: undercoat layer
3: charge generation layer
4: charge transport layer
5: photosensitive layer
10A: photoreceptor
10B: photoreceptor
7: electrophotographic photoreceptor
8: charging device
9: exposure device
11: developing device
13: cleaning device
14: lubricant
40: transfer device
50: intermediate transfer member
100: image forming apparatus
120: image forming apparatus
131: cleaning blade
132: fibrous member (roll shape)
133: fibrous member (flat brush shape)
300: process cartridge

## Claims

1. An electrophotographic photoreceptor comprising:
an outermost layer that contains a charge transport material and a binder resin,
wherein the binder resin includes a polyester resin P_{A} having an elastic deformation rate X_{A} of 53.0% or greater and a polycarbonate resin P_{B} having an elastic deformation rate X_{B} that is less than the elastic deformation rate X_{A} of the polyester resin P_{A} by a range of 5% or greater and 12% or less. The elastic deformation rate is determined according to the method detailed in the description.

2. The electrophotographic photoreceptor according to claim 1,
wherein a content ratio (polyester resin P_{A}:Polycarbonate resin P_{B}) of the polyester resin P_{A} to the polycarbonate resin P_{B} is in a range of 7:3 to 3:7 in terms of a mass.

3. The electrophotographic photoreceptor according to claim 2,
wherein the content ratio (polyester resin P_{A}:Polycarbonate resin P_{B}) of the polyester resin P_{A} to the polycarbonate resin P_{B} is in a range of 7:3 to 5:5 in terms of the mass.

4. The electrophotographic photoreceptor according to any one of claims 1 to 3,
wherein the polyester resin P_{A} includes a polyester resin having a dicarboxylic acid unit (A) represented by Formula (A) and a diol unit (B) represented by Formula (B),
in Formula (A), Ar^{A1} and Ar^{A2} each independently represent an aromatic ring that may have a substituent, L^{A} represents a single bond or a divalent linking group, and n^{A1} represents 0, 1, or 2,
in Formula (B), Ar^{B1} and Ar^{B2} each independently represent an aromatic ring that may have a substituent, L^{B} represents a single bond, an oxygen atom, a sulfur atom, or -C(Rb¹)(Rb²)-, n^{B1} represents 0, 1, or 2, Rb¹ and Rb² each independently represent a hydrogen atom, an alkyl group having 1 or more and 20 or less carbon atoms, an aryl group having 6 or more and 12 or less carbon atoms, or an aralkyl group having 7 or more and 20 or less carbon atoms, and Rb¹ and Rb² may be bonded to each other to form a cyclic alkyl group.

5. The electrophotographic photoreceptor according to any one of claims 1 to 4,
wherein the polycarbonate resin P_{B} includes a polycarbonate resin having a constitutional unit represented by Formula (PCA) and a constitutional unit represented by Formula (PCB),
in Formula (PCA), R^{P1} and R^{P2} each independently represent a hydrogen atom, a halogen atom, an alkyl group having 1 or more and 6 or less carbon atoms, a cycloalkyl group having 5 or more and 7 or less carbon atoms, or an aryl group having 6 or more and 12 or less carbon atoms,
in Formula (PCB), R^{P3} and R^{P4} each independently represent a hydrogen atom, a halogen atom, an alkyl group having 1 or more and 6 or less carbon atoms, a cycloalkyl group having 5 or more and 7 or less carbon atoms, or an aryl group having 6 or more and 12 or less carbon atoms, and X^{P1} represents a phenylene group, a biphenylene group, a naphthylene group, a linear or branched alkylene group, or a cycloalkylene group.

6. A process cartridge comprising:
the electrophotographic photoreceptor according to any one of claims 1 to 5,
wherein the process cartridge is attachable to and detachable from an image forming apparatus.

7. An image forming apparatus comprising:
the electrophotographic photoreceptor according to any one of claims 1 to 5;
a charging device that comes into direct contact with a surface of the electrophotographic photoreceptor and applies only a DC voltage to charge the surface of the electrophotographic photoreceptor;
an electrostatic latent image forming device that forms an electrostatic latent image on the charged surface of the electrophotographic photoreceptor;
a developing device that develops the electrostatic latent image formed on the surface of the electrophotographic photoreceptor with a developer containing a toner to form a toner image; and
a transfer device that transfers the toner image to a surface of a recording medium.

8. The image forming apparatus according to claim 7,
wherein the charging device includes a charging member that charges the surface of the electrophotographic photoreceptor and a DC voltage application unit that applies only the DC voltage to the charging member, and
a voltage applied to the charging member from the DC voltage application unit is -700 V or greater and -300 V or less.

## Patentansprüche

1. Elektrophotographischer Photorezeptor, umfassend:
eine äußerste Schicht, die ein Ladungstransportmaterial und ein Bindemittelharz enthält,
wobei das Bindemittelharz ein Polyesterharz P_{A} mit einer elastischen Verformungsrate X_{A} von 53,0 % oder mehr und ein Polycarbonatharz P_{B} mit einer elastischen Verformungsrate X_{B}, die um einen Bereich von 5 % oder mehr und 12 % oder weniger kleiner als die elastische Verformungsrate X_{A} des Polyesterharzes P_{A} ist, enthält. Die elastische Verformungsrate wird gemäß dem in der Beschreibung detaillierten Verfahren bestimmt.

2. Elektrophotographischer Photorezeptor nach Anspruch 1,
wobei ein Gehaltsverhältnis (Polyesterharz P_{A}:Polycarbonatharz P_{B}) des Polyesterharzes P_{A} zu dem Polycarbonatharz P_{B} in einem Bereich von 7:3 bis 3:7 in Bezug auf eine Masse liegt.

3. Elektrophotographischer Photorezeptor nach Anspruch 2,
wobei das Gehaltsverhältnis (Polyesterharz P_{A}:Polycarbonatharz P_{B}) des Polyesterharzes P_{A} zu dem Polycarbonatharz P_{B} in einem Bereich von 7:3 bis 5:5 in Bezug auf die Masse liegt.

4. Elektrophotographischer Photorezeptor nach einem der Ansprüche 1 bis 3, wobei das Polyesterharz P_{A} ein Polyesterharz, das eine Dicarbonsäureeinheit (A), die durch Formel (A) dargestellt wird, und eine Diol-Einheit (B), die durch Formel (B) dargestellt wird, enthält, enthält,
in Formel (A) Ar^{A1} und Ar^{A2} jeweils unabhängig voneinander einen aromatischen Ring, der einen Substituenten aufweisen kann, darstellen, L^{A} eine Einfachbindung oder eine divalente Verknüpfungsgruppe darstellt und n^{A1} 0, 1 oder 2 darstellt,
in Formel (B) Ar^{B1} und Ar^{B2} jeweils unabhängig voneinander einen aromatischen Ring, der einen Substituenten aufweisen kann, darstellen, L^{B} eine Einfachbindung, ein Sauerstoffatom, ein Schwefelatom oder -C(Rb¹)(Rb²)- darstellt, n^{B1} 0, 1 oder 2 darstellt, Rb¹ und Rb² jeweils unabhängig voneinander ein Wasserstoffatom, eine Alkylgruppe mit 1 oder mehr und 20 oder weniger Kohlenstoffatomen, eine Arylgruppe mit 6 oder mehr und 12 oder weniger Kohlenstoffatomen oder eine Aralkylgruppe mit 7 oder mehr und 20 oder weniger Kohlenstoffatomen darstellen und Rb¹ und Rb² miteinander gebunden sein können, um eine zyklische Alkylgruppe zu bilden.

5. Elektrophotographischer Photorezeptor nach einem der Ansprüche 1 bis 4, wobei das Polycarbonatharz P_{B} ein Polycarbonatharz, das eine durch Formel (PCA) dargestellte Konstitutionseinheit und eine durch Formel (PCB) dargestellte Konstitutionseinheit enthält, enthält,
in Formel (PCA) R^{P1} und R^{P2} jeweils unabhängig voneinander ein Wasserstoffatom, ein Halogenatom, eine Alkylgruppe mit 1 oder mehr und 6 oder weniger Kohlenstoffatomen, eine Cycloalkylgruppe mit 5 oder mehr und 7 oder weniger Kohlenstoffatomen oder eine Arylgruppe mit 6 oder mehr und 12 oder weniger Kohlenstoffatomen darstellen,
in Formel (PCB) R^{P3} und R^{P4} jeweils unabhängig voneinander ein Wasserstoffatom, ein Halogenatom, eine Alkylgruppe mit 1 oder mehr und 6 oder weniger Kohlenstoffatomen, eine Cycloalkylgruppe mit 5 oder mehr und 7 oder weniger Kohlenstoffatomen oder eine Arylgruppe mit 6 oder mehr und 12 oder weniger Kohlenstoffatomen darstellen und X^{P1} eine Phenylen-Gruppe, eine Biphenylen-Gruppe, eine Naphthylen-Gruppe, eine lineare oder verzweigte Alkylengruppe oder eine Cycloalkylengruppe darstellt.

6. Prozesskartusche, umfassend:
den elektrophotographischen Photorezeptor nach einem der Ansprüche 1 bis 5,
wobei die Prozesskartusche an einer Bilderzeugungsvorrichtung anbringbar und von dieser lösbar ist.

7. Bilderzeugungsvorrichtung, umfassend:
den elektrophotographischen Photorezeptor nach einem der Ansprüche 1 bis 5;
eine Ladevorrichtung, die mit einer Oberfläche des elektrophotographischen Photorezeptors in direkten Kontakt kommt und nur eine Gleichstromspannung anlegt, um die Oberfläche des elektrophotographischen Photorezeptors zu laden;
eine Erzeugungsvorrichtung für elektrostatisches Latentbild, die ein elektrostatisches Latentbild auf der geladenen Oberfläche des elektrophotographischen Photorezeptors erzeugt;
eine Entwicklungsvorrichtung, die das elektrostatische Latentbild, das auf der Oberfläche des elektrophotographischen Photorezeptors erzeugt wird, mit einem Entwickler, der einen Toner enthält, entwickelt, um ein Tonerbild zu erzeugen; und
eine Übertragungsvorrichtung, die das Tonerbild auf eine Oberfläche eines Aufzeichnungsmediums überträgt.

8. Bilderzeugungsvorrichtung nach Anspruch 7,
wobei die Ladevorrichtung ein Ladeelement, das die Oberfläche des elektrophotographischen Photorezeptors lädt, und eine Gleichstromspannungs-Anlegeeinheit, die nur die Gleichstromspannung an das Ladeelement anlegt, enthält, und
eine an das Ladeelement von der Gleichstromspannungs-Anlegeeinheit angelegte Spannung -700 V oder größer und -300 V oder kleiner ist.

## Revendications

1. Photorécepteur électrophotographique comprenant :
une couche la plus externe qui contient un matériau de transport de charge et une résine liante,
dans lequel la résine liante inclut une résine polyester P_{A} ayant un taux de déformation élastique X_{A} de 53,0 % ou plus et une résine polycarbonate P_{B} ayant un taux de déformation élastique X_{B} qui est inférieur au taux de déformation élastique X_{A} de la résine polyester P_{A} d'une plage de 5 % ou plus et 12 % ou moins. Le taux de déformation élastique est déterminé selon la méthode détaillée dans la description.

2. Photorécepteur électrophotographique selon la revendication 1,
dans lequel un rapport de teneur (résine polyester P_{A} : résine polycarbonate P_{B}) de la résine polyester P_{A} à la résine polycarbonate P_{B} est dans une plage de 7:3 à 3:7 en termes de masse.

3. Photorécepteur électrophotographique selon la revendication 2,
dans lequel le rapport de teneur (résine polyester P_{A} : résine polycarbonate P_{B}) de la résine polyester P_{A} à la résine polycarbonate P_{B} est dans une plage de 7:3 à 5:5 en termes de masse.

4. Photorécepteur électrophotographique selon l'une quelconque des revendications 1 à 3, dans lequel la résine polyester P_{A} inclut une résine polyester ayant une unité d'acide dicarboxylique (A) représentée par Formule (A) et une unité de diol (B) représentée par Formule (B),
dans Formule (A), Ar^{A1} et Ar^{A2} représentent chacun indépendamment un cycle aromatique qui peut avoir un substituant, L^{A} représente une liaison simple ou un groupe de liaison divalent, et n^{A1} représente 0, 1 ou 2,
dans Formule (B), Ar^{B1} et Ar^{B2} représentent chacun indépendamment un cycle aromatique qui peut avoir un substituant, L^{B} représente une liaison simple, un atome d'oxygène, un atome de soufre ou -C(Rb¹)(Rb²)-, n^{B1} représente 0, 1 ou 2, Rb¹ et Rb² représentent chacun indépendamment un atome d'hydrogène, un groupe alkyle ayant 1 ou plus et 20 ou moins atomes de carbone, un groupe aryle ayant 6 ou plus et 12 ou moins atomes de carbone, ou un groupe aralkyle ayant 7 ou plus et 20 ou moins atomes de carbone, et Rb¹ et Rb² peuvent être liés l'un à l'autre pour former un groupe alkyle cyclique.

5. Photorécepteur électrophotographique selon l'une quelconque des revendications 1 à 4, dans lequel la résine polycarbonate P_{B} inclut une résine polycarbonate ayant une unité constitutive représentée par Formule (PCA) et une unité constitutive représentée par Formule (PCB),
dans Formule (PCA), R^{P1} et R^{P2} représentent chacun indépendamment un atome d'hydrogène, un atome d'halogène, un groupe alkyle ayant 1 ou plus et 6 ou moins atomes de carbone, un groupe cycloalkyle ayant 5 ou plus et 7 ou moins atomes de carbone, ou un groupe aryle ayant 6 ou plus et 12 ou moins atomes de carbone,
dans Formule (PCB), R^{P3} et R^{P4} représentent chacun indépendamment un atome d'hydrogène, un atome d'halogène, un groupe alkyle ayant 1 ou plus et 6 ou moins atomes de carbone, un groupe cycloalkyle ayant 5 ou plus et 7 ou moins atomes de carbone, ou un groupe aryle ayant 6 ou plus et 12 ou moins atomes de carbone, et X^{P1} représente un groupe phénylène, un groupe biphénylène, un groupe naphtylène, un groupe alkylène linéaire ou ramifié, ou un groupe cycloalkylène.

6. Cartouche de traitement comprenant :
le photorécepteur électrophotographique selon l'une quelconque des revendications 1 à 5,
dans laquelle la cartouche de traitement peut être fixée à un appareil de formation d'images et en être détachée.

7. Appareil de formation d'images comprenant :
le photorécepteur électrophotographique selon l'une quelconque des revendications 1 à 5 ;
un dispositif de charge qui entre en contact direct avec une surface du photorécepteur électrophotographique et applique uniquement une tension continue pour charger la surface du photorécepteur électrophotographique ;
un dispositif de formation d'images latentes électrostatiques qui forme une image latente électrostatique sur la surface chargée du photorécepteur électrophotographique ;
un dispositif de développement qui développe l'image latente électrostatique formée sur la surface du photorécepteur électrophotographique avec un révélateur contenant un toner pour former une image de toner ; et
un dispositif de transfert qui transfère l'image de toner sur une surface d'un support d'enregistrement.

8. Appareil de formation d'images selon la revendication 7,
dans lequel le dispositif de charge inclut un élément de charge qui charge la surface du photorécepteur électrophotographique et une unité d'application de tension continue qui applique uniquement la tension continue à l'élément de charge, et
une tension appliquée à l'élément de charge à partir de l'unité d'application de tension continue est de -700 V ou plus et de -300 V ou moins.
